



US008454454B2

(12) **United States Patent**  
Sullivan et al.

(10) **Patent No.:** US 8,454,454 B2  
(45) **Date of Patent:** \*Jun. 4, 2013

(54) **GOLF BALL HAVING REDUCED SURFACE HARDNESS**

(75) Inventors: **Michael J. Sullivan**, Barrington, RI (US); **Mark L. Binette**, Mattapoisett, MA (US); **Brian Comeau**, Berkley, MA (US)

(73) Assignee: **Acushnet Company**, Fairhaven, MA (US)

(\*) Notice: Subject to any disclaimer, the term of this patent is extended or adjusted under 35 U.S.C. 154(b) by 596 days.

This patent is subject to a terminal disclaimer.

(21) Appl. No.: **12/695,379**

(22) Filed: **Jan. 28, 2010**

(65) **Prior Publication Data**

US 2010/0173726 A1 Jul. 8, 2010

**Related U.S. Application Data**

(63) Continuation-in-part of application No. 12/395,023, filed on Feb. 27, 2009, now Pat. No. 7,819,760, which is a continuation of application No. 12/394,942, filed on Feb. 27, 2009, which is a continuation-in-part of application No. 12/056,457, filed on Mar. 27, 2008, now Pat. No. 7,678,313, which is a continuation of application No. 12/048,665, filed on Mar. 14, 2008, now Pat. No. 7,678,312, which is a continuation-in-part of application No. 11/772,903, filed on Jul. 3, 2007, now Pat. No. 7,537,529, application No. 12/695,379, which is a continuation-in-part of application No. 12/342,545, filed on Dec. 23, 2008, now Pat. No. 7,946,934, which is a continuation-in-part of application No. 12/339,495, filed on Dec. 19, 2008, now Pat. No.

7,815,526, which is a continuation-in-part of application No. 12/196,522, filed on Aug. 22, 2008, now Pat. No. 7,582,025, which is a continuation of application No. 11/939,635, filed on Nov. 14, 2007, now Pat. No. 7,427,242.

(51) **Int. Cl.**  
**A63B 37/06** (2006.01)

(52) **U.S. Cl.**  
USPC ..... 473/374

(58) **Field of Classification Search**  
USPC ..... 473/376, 373, 374  
See application file for complete search history.

(56) **References Cited**

**U.S. PATENT DOCUMENTS**

|               |         |                              |
|---------------|---------|------------------------------|
| 3,784,209 A   | 1/1974  | Berman                       |
| 3,986,802 A   | 10/1976 | Isom                         |
| 4,570,937 A   | 2/1986  | Yamada                       |
| 4,650,193 A * | 3/1987  | Molitor et al. ..... 473/373 |
| 5,033,748 A   | 7/1991  | Ebisuno                      |
| 5,334,673 A   | 8/1994  | Wu                           |
| 5,484,870 A   | 1/1996  | Wu                           |
| 5,516,110 A   | 5/1996  | Yabuki et al.                |
| 5,697,856 A   | 12/1997 | Moriyama et al.              |
| 5,733,206 A   | 3/1998  | Nesbitt et al.               |
| 5,782,707 A   | 7/1998  | Yamagishi et al.             |

(Continued)

*Primary Examiner* — Raeann Gorden

(74) *Attorney, Agent, or Firm* — Margaret C. Barker

(57) **ABSTRACT**

A golfball comprising a core and a cover, the core comprising an outer surface and a geometric center, the outer surface being treated with and comprising a fatty acid and/or fatty acid salt composition, the outer surface further having a first hardness and the geometric center having a second hardness, wherein the first hardness is the same as or different than the second hardness.

**14 Claims, 4 Drawing Sheets**



## U.S. PATENT DOCUMENTS

|              |         |                  |                 |         |                              |
|--------------|---------|------------------|-----------------|---------|------------------------------|
| 5,803,834 A  | 9/1998  | Yamagishi et al. | 6,689,860 B2    | 2/2004  | Iwami                        |
| 5,957,784 A  | 9/1999  | Asakura et al.   | 6,739,986 B2    | 5/2004  | Higuchi et al.               |
| 5,976,443 A  | 11/1999 | Nesbitt et al.   | 6,805,644 B1    | 10/2004 | Moriyama et al.              |
| 6,113,831 A  | 9/2000  | Nesbitt et al.   | 6,815,521 B2    | 11/2004 | Iwami                        |
| 6,319,154 B1 | 11/2001 | Yoshida et al.   | 6,835,794 B2    | 12/2004 | Wu et al.                    |
| 6,417,278 B1 | 7/2002  | Ladd et al.      | 6,837,803 B2    | 1/2005  | Nanba et al.                 |
| 6,432,342 B1 | 8/2002  | Nesbitt et al.   | 6,921,345 B2    | 7/2005  | Higuchi et al.               |
| 6,458,895 B1 | 10/2002 | Wrigley et al.   | 6,932,720 B2    | 8/2005  | Hogge et al.                 |
| 6,494,793 B1 | 12/2002 | Ohama            | 7,004,854 B2    | 2/2006  | Hogge et al.                 |
| 6,494,794 B1 | 12/2002 | Ohama            | 7,153,224 B2    | 12/2006 | Higuchi et al.               |
| 6,506,851 B2 | 1/2003  | Wu               | 7,182,702 B2    | 2/2007  | Hogge et al.                 |
| 6,533,683 B2 | 3/2003  | Watanabe         | 7,819,760 B2 *  | 10/2010 | Sullivan et al. .... 473/373 |
| 6,537,158 B2 | 3/2003  | Watanabe         | 8,047,932 B2 *  | 11/2011 | Sullivan et al. .... 473/373 |
| 6,632,147 B2 | 10/2003 | Cavallaro et al. | 2003/0209840 A1 | 11/2003 | Hogge et al.                 |
| 6,635,716 B2 | 10/2003 | Voorheis et al.  | 2003/0236135 A1 | 12/2003 | Hogge et al.                 |
| 6,659,888 B2 | 12/2003 | Endo et al.      | 2005/0176523 A1 | 8/2005  | Boehm et al.                 |
| 6,679,791 B2 | 1/2004  | Watanabe         |                 |         |                              |

\* cited by examiner



FIG. 1



FIG. 2



FIG. 3A



FIG. 3B



FIG. 4A



FIG. 4B

## GOLF BALL HAVING REDUCED SURFACE HARDNESS

### CROSS-REFERENCE TO RELATED APPLICATIONS

This application is a continuation-in-part of U.S. patent application Ser. No. 12/395,023, filed Feb. 27, 2009, now U.S. Pat. No. 7,819,760, which is a continuation of U.S. patent application Ser. No. 12/394,942, filed Feb. 27, 2009, which is a continuation-in-part of U.S. patent application Ser. No. 12/056,457, filed Mar. 27, 2008, now U.S. Pat. No. 7,678,313, which is a continuation of U.S. patent application Ser. No. 12/048,665, filed Mar. 14, 2008, now U.S. Pat. No. 7,678,312, which is a continuation-in-part of U.S. patent application Ser. No. 11/772,903, filed Jul. 3, 2007, now U.S. Pat. No. 7,537,529. This application is also a continuation-in-part of U.S. patent application Ser. No. 12/342,545, filed Dec. 23, 2008, now U.S. Pat. No. 7,946,934, which is a continuation-in-part of U.S. patent application Ser. No. 12/339,495, filed Dec. 19, 2008, now U.S. Pat. No. 7,815,526, which is a continuation-in-part of U.S. patent application Ser. No. 12/196,522, filed Aug. 22, 2008, now U.S. Pat. No. 7,582,025, which is a continuation of U.S. patent application Ser. No. 11/939,635, filed Nov. 14, 2007, now U.S. Pat. No. 7,427,242. The disclosures of the parent cases are incorporated by reference herein in their entireties.

### FIELD OF THE INVENTION

This invention relates generally to golf balls with cores, more particularly either single layer cores or multilayer cores, having a surface hardness equal to or less than the center hardness.

### BACKGROUND OF THE INVENTION

Solid golf balls are typically made with a solid core encased by a cover, both of which can have multiple layers, such as a dual core having a solid center and an outer core layer, or a multi-layer cover having an inner and outer cover layer. Generally, golf ball cores and/or centers are constructed with a thermoset rubber, typically a polybutadiene-based composition. The cores are usually heated and crosslinked to create certain characteristics, such as higher or lower compression, which can impact the spin rate of the ball and/or provide better “feel.” These and other characteristics can be tailored to the needs of golfers of different abilities. From the perspective of a golf ball manufacturer, it is desirable to have cores exhibiting a wide range of properties, such as resilience, durability, spin, and “feel;” because this enables the manufacturer to make and sell many different types of golf balls suited to differing levels of ability.

Heretofore, most single core golf ball cores have had a conventional hard-to-soft hardness gradient from the surface of the core to the center of the core. The patent literature contains a number of references that discuss a hard surface to soft center hardness gradient across a golf ball core.

U.S. Pat. No. 4,650,193 to Molitor et al. generally discloses a hardness gradient in the surface layers of a core by surface treating a slug of curable elastomer with a cure-altering agent and subsequently molding the slug into a core. This treatment allegedly creates a core with two zones of different compositions, the first part being the hard, resilient, central portion of the core, which was left untreated, and the second being the soft, deformable, outer layer of the core, which was treated by the cure-altering agent. The two “layers” or regions of the

core are integral with one another and, as a result, achieve the effect of a gradient of soft surface to hard center.

U.S. Pat. No. 3,784,209 to Berman, et al. generally discloses a soft-to-hard hardness gradient. The '209 patent discloses a non-homogenous, molded golf ball with a core of “mixed” elastomers. A center sphere of uncured elastomeric material is surrounded by a compatible but different uncured elastomer. When both layers of elastomer are concurrently exposed to a curing agent, they become integral with one another, thereby forming a mixed core. The center of this core, having a higher concentration of the first elastomeric material, is harder than the outer layer. One drawback to this method of manufacture is the time-consuming process of creating first elastomer and then a second elastomer and then molding the two together.

Other patents discuss cores that receive a surface treatment to provide a soft ‘skin’. However, since the interior portions of these cores are untreated, they have the similar hard surface to soft center gradient as conventional cores. For example, U.S. Pat. No. 6,113,831 to Nesbitt et al. generally discloses a conventional core and a separate soft skin wrapped around the core. This soft skin is created by exposing the preform slug to steam during the molding process so that a maximum mold temperature exceeds a steam set point, and by controlling exothermic molding temperatures during molding. The skin comprises the radially-outermost  $\frac{1}{32}$  inch to  $\frac{1}{4}$  inch of the spherical core. U.S. Pat. Nos. 5,976,443 and 5,733,206, both to Nesbitt et al., disclose the addition of water mist to the outside surface of the slug before molding in order to create a soft skin. The water allegedly softens the compression of the core by retarding crosslinking on the core surface, thereby creating an even softer soft skin around the hard central portion.

Additionally, a number of patents disclose multilayer golf ball cores, where each core layer has a different hardness thereby creating a hardness gradient from core layer to core layer.

There remains a need, however, for an improved and inexpensively manufactured single layer or multilayer core which exhibits a soft-to-hard gradient (a “negative” gradient) between the core outer surface and any or all of the core geometric center, core layer region(s) and core layer(s). A core exhibiting such characteristics would allow the golf ball designer to create and provide products with unique combinations of desired compression, “feel,” and spin.

### BRIEF DESCRIPTION OF THE DRAWINGS

FIG. 1 is a schematic cross section illustrating one embodiment of the golf ball of the present invention;

FIG. 2 is a schematic cross section illustrating another embodiment of the golf ball of the present invention;

FIGS. 3A and 3B are schematic cross sections illustrating still another embodiment of the golf ball of the present invention; and

FIGS. 4A and 4B are schematic cross sections illustrating yet another embodiment of the golf ball of the present invention.

### SUMMARY OF THE INVENTION

The present invention provides a golf ball comprising a core and a cover wherein the core comprises an outer surface and a geometric center, the outer surface being treated with and comprising a fatty acid and/or fatty acid salt composition. The outer surface has a first hardness and the geometric center

has a second hardness wherein the first hardness is less than the second hardness to define a negative hardness gradient.

In one embodiment, the core comprises a thermoset rubber composition. The thermoset rubber composition may comprise a polybutadiene material and/or have a surface hardness of about 50 Shore C or greater. In another embodiment, the polybutadiene composition is at least partially crosslinked.

The at least one fatty acid and/or fatty acid salt composition may comprise oleic acid, palmitic acid, stearic acid, behenic acid, pelargonic acid, linoleic acid, linolenic acid, arachidonic acid, caproic acid, caprylic acid, capric acid, lauric acid, erucic acid, myristic acid, benzoic acid, phenylacetic acid, or naphthalenoic acid.

The at least one fatty acid and/or fatty acid salt composition may comprise a cation selected from the group comprising barium, lithium, sodium, zinc, bismuth, chromium, cobalt, copper, potassium, strontium, titanium, tungsten, magnesium, cesium, iron, nickel, silver, aluminum, tin and calcium.

The at least one fatty acid and/or fatty acid salt composition may further comprise at least one of an antioxidant, a sulfur-bearing compound, zinc methacrylate, zinc dimethacrylate, a softening acrylate monomer or oligomer, a thermoplastic resin, or an hydroquinone.

The thermoplastic resin may comprise at least one of polyethylene vinyl acetate, polyethylene butyl acrylate, polyethylene methyl acrylate, polyethylene acrylic acid, polyethylene methacrylic acid or an ionomer.

An intermediate core layer may be disposed about the core and adjacent the cover layer.

In another embodiment, the golf ball comprises a core and a cover. The core comprises an outer surface and a geometric center. The outer surface comprises a fatty acid and/or fatty acid salt composition and has a first hardness and the geometric center has a second hardness greater than the first hardness to define a negative hardness gradient.

In a further embodiment, the golf ball comprises a core and at least one cover layer disposed about the core. The core comprises a geometric center and an outer surface. The core further comprises an untreated region extending radially from the geometric center a predetermined distance  $D_{UTr}$ . A treated region is disposed about the untreated region and extends inward from the outer surface a predetermined depth  $D_{Tr}$ . The untreated region and the treated region are adjacent each other and concentric with the geometric center. The treated region has been exposed to and comprises a fatty acid and/or fatty acid salt composition. The treated region comprises a first hardness and the untreated region comprises a second hardness different than the first hardness.

In one embodiment, the first hardness is less than the second hardness. In additional embodiments, the first hardness may be greater than or the same as the second hardness. These additional embodiments may occur where, for example, the hardness of the treated region was greater than the hardness of the untreated region prior to being treated with the fatty acid and/or fatty acid salt composition. Or, it may occur where the fatty acid/fatty acid salt treated and comprising region further comprises materials/compositions including but not limited to zinc methacrylate, zinc dimethacrylate, a thermoplastic resin, an hydroquinone, and/or peroxide which tend to harden the fatty acid and/or fatty acid salt treated and comprising surface or region. Meanwhile, however, an improved golf ball is provided over golf balls which have not been treated with nor comprise a fatty acid and/or fatty acid salt composition as in the present invention.

The golf ball core may further comprise an intermediate untreated region disposed about the untreated region and adjacent the treated region, said intermediate untreated region

comprising a third hardness wherein the first hardness is greater than the second hardness and less than the third hardness.

Alternatively, the golf ball core may further comprise an intermediate untreated region disposed about the untreated region and adjacent the treated region, said intermediate untreated region comprising a third hardness wherein the first hardness is less than the second hardness and the third hardness.

10 The golf ball core may comprise an intermediate untreated region disposed about the untreated region and adjacent the treated region, said intermediate untreated region comprising a third hardness wherein the first hardness is greater than the second hardness and the third hardness.

15 The golf ball core may comprise an intermediate untreated region disposed about the untreated region and adjacent the treated region, said intermediate untreated region comprising a third hardness wherein the first hardness is greater than the second hardness and substantially similar to the third hardness.

20 In still another embodiment, the golf ball comprises a core and at least one cover layer disposed about the core. The core comprises a geometric center and an outer surface. The core further comprises an untreated region extending radially from the geometric center a distance  $D_{UTr}$ . A treated region is disposed about the untreated region and extends inward from the outer surface a depth  $D_{Tr}$ . The treated region has been exposed to and comprises a fatty acid and/or fatty acid salt composition. The treated region comprises a first hardness and the untreated region comprises a second hardness wherein the first hardness is different than the second hardness.

25 In yet another embodiment, the golf ball comprises a core and at least one cover layer disposed about the core. The core comprises a geometric center and an outer surface. The core further comprises an untreated region which extends radially from the geometric center a distance  $D_{UTr}$ . Additionally, treated region is disposed about the untreated region and extends inward from the outer surface a depth  $D_{Tr}$ . The treated region has been exposed to and comprises a fatty acid and/or fatty acid salt composition. Furthermore, the core comprises an intermediate untreated region disposed about the untreated region and adjacent the treated region. The intermediate untreated region has a third hardness, wherein the first hardness is different than the second hardness and the third hardness.

30 The core may comprise a single layer core comprising the untreated region, the intermediate untreated region and the treated region.

35 The core may comprise a multilayer core comprising a first core layer extending radially from the geometric center and a second core layer disposed about the first core layer, wherein the first core layer comprises the untreated region and the second core layer comprises the treated region. The treated region may alternatively occupy not only the second core layer but also extend into a region within the first core layer adjacent the second core layer.

40 Further, the core may comprise a first core layer extending radially from the geometric center and a second core layer disposed about the first core layer, wherein the first core layer comprises the untreated region and an intermediate untreated region, and the second core layer comprises the treated region.

45 The core may also comprise a first core layer extending radially from the geometric center, a second core layer disposed about the first core layer and a third core layer disposed about the second core layer, wherein the first core layer com-

prises the untreated region, wherein the second core layer comprises the intermediate untreated region, and wherein the third core layer comprises the treated region.

The present invention is also directed to a golf ball comprising a core and a cover wherein the core comprises a geometric center and a treated outer surface, the treated outer surface having a first hardness and the geometric center having a second hardness, the treated outer surface being treated with a surface-softening material comprising at least one fatty acid and/or fatty acid salt composition such that the second hardness is greater than the first hardness to define a negative hardness gradient.

In another embodiment, the golf ball comprising a core and a cover, the core comprising a geometric center and an outer surface, the outer surface comprising fatty acid and/or fatty acid salt composition, the geometric center having a hardness ( $H_g$ ) and the outer surface having an extrapolated hardness ( $H_E$ ) and an actual hardness ( $H_{OS}$ ) wherein  $H_E$  is derived from a five point extrapolation within three quarters of an outer core diameter and  $H_{OS}$  as measured on the curved surface of the core, and the cover has a hardness ( $H_C$ ), wherein  $H_C > H_E > H_g > H_{OS}$ .

Also, the present invention may be directed to a golf ball comprising a core and a cover, the core comprising a geometric center and an outer surface, the outer surface comprising fatty acid and/or fatty acid salt composition, the geometric center having a hardness ( $H_g$ ) and the outer surface having an extrapolated hardness ( $H_E$ ) and an actual hardness ( $H_{OS}$ ) wherein  $H_E$  is derived from a five point extrapolation within three quarters of an outer core diameter and  $H_{OS}$  as measured on the curved surface of the core, and the cover has a hardness ( $H_C$ ), wherein  $H_C < H_E > H_g > H_{OS}$ .

The golf ball may advantageously comprise a thermoset rubber composition core and a cover, said core comprising an outer surface and a geometric center, the outer surface having a treated region comprising a fatty acid and/or fatty acid salt composition extending inward from the outer surface from about 0.001 inches to about 0.200 inches, the treated region further having a first hardness and the geometric center having a second hardness, wherein the first hardness is less than the second hardness to define a negative hardness gradient.

Additionally, the golf ball may comprise a core and a cover, said core comprising a fatty acid and/or fatty acid salt composition outer surface and a geometric center, the fatty acid and/or fatty acid salt composition outer surface having a first hardness and the geometric center having a second hardness wherein the first hardness is less than the second hardness to define a negative hardness gradient.

Moreover, the golf ball may comprise a core and a cover, the core comprising an outer surface and a geometric center, the outer surface being treated with a fatty acid and/or fatty acid salt composition, the outer surface having a hardness that is less than a hardness of the geometric center to define a negative hardness gradient.

In any embodiment, each core region and core layer may radially extend from the geometric center and be concentric with the geometric center. Similarly, the core outer surface may be concentric with the geometric center.

As discussed more fully below, the fatty acid and/or fatty acid salt composition acts as a plasticizer to soften the treated core surface and become intimately mixed therewith.

The present invention is directed to a method of making a golf ball comprising the steps of providing an untreated golf ball core comprising a thermoset rubber composition, the untreated golf ball core comprising an untreated outer surface having a hardness; treating the untreated outer surface of the untreated golf ball core with a surface-softening material

comprising at least one fatty acid or fatty acid salt composition to form a golf ball core comprising a treated outer surface having a hardness less than the hardness of the untreated outer surface; and foaming at least one cover layer about the core to form the golf ball.

Further, the present invention is directed to a method of making a golf ball comprising the steps of providing an untreated golf ball core comprising a thermoset rubber composition, said untreated golf ball core comprising a geometric center and an untreated outer surface, each having a hardness; treating the untreated golf ball core with a surface-softening material comprising at least one fatty acid or fatty acid salt composition to form a golf ball core comprising a treated outer surface having a hardness less than the hardness of the untreated outer surface, the treated outer surface further having a surface hardness less than the hardness of the geometric center of the untreated golf ball core to define a negative hardness gradient; and forming a cover layer about the core to form the golf ball.

In an alternative embodiment, the invention is directed to a method of making a golf ball comprising the steps of providing a preform comprising an uncured polybutadiene composition; coating the preform with a first surface-softening material comprising at least one of a fatty acid compound or a fatty acid salt compound; curing the coated preform at a predetermined temperature to form a crosslinked golf ball core having an outer surface having a first hardness and a geometric center having a second hardness greater than the first to define a negative hardness gradient; and forming a cover layer about the core to form the golf ball.

Additionally, the present invention is directed to a method of making a golf ball comprising the steps of: extruding a polybutadiene composition to form a cylindrical extrudate; cutting the extrudate to form an uncured polybutadiene preform; uniformly coating the preform with a surface-softening material comprising at least one fatty acid or fatty acid salt composition; curing the coated preform to form a crosslinked core having an outer surface having a first hardness and a geometric center having a second hardness greater than the first to define a negative hardness gradient; centerless-grinding the cured core to form a uniformly-spherical core having increased surface roughness; forming an inner cover layer about the uniformly-spherical core; and forming an outer cover layer about the inner cover layer to form the golf ball.

Alternatively, the golf ball comprises several layers which are treated with a surface-softening material comprising at least one fatty acid or fatty acid salt composition or blends/combinations thereof.

The present invention is also directed to a golf ball comprising a core and a cover, wherein the core has an outer

surface that is treated with a surface-softening material comprising at least one fatty acid or fatty acid salt composition

such that the outer surface has a hardness ratio (R) of the hardness after treatment ( $H_2$ ) to the hardness before treatment

( $H_1$ ) of less than about 0.95.

The invention is further directed to a golf ball comprising a core and a cover, wherein the core has a geometric center having a hardness ( $H_g$ ) and the core has an outer surface that is treated with a surface-softening material comprising at least one fatty acid or fatty acid salt composition such that the outer surface has an extrapolated hardness ( $H_E$ ) and an actual hardness ( $H_{OS}$ ) wherein  $H_E$  is derived from a five point extrapolation within three quarters of an outer core diameter and  $H_{OS}$  is measured on the curved surface of the core, and the cover has a hardness ( $H_C$ ), wherein  $H_C > H_E > H_g > H_{OS}$ .

In still another embodiment, a golf ball comprises a core and a cover, wherein the core has a geometric center having a

hardness ( $H_g$ ) and the core has an outer surface that is treated with at least one fatty acid or fatty acid salt such that the outer surface has an extrapolated hardness ( $H_E$ ) and an actual hardness ( $H_{OS}$ ) wherein  $H_E$  is derived from a five point extrapolation within three quarters of an outer core diameter and  $H_{OS}$  is measured on the curved surface of the core, and the cover has a hardness ( $H_C$ ), wherein  $H_E > H_g > H_{OS} > H_C$ .

An advantage of the present invention is that a core is formed having a hardness gradient between the core treated outer surface comprising the fatty acid and/or fatty acid salt composition and the untreated regions within the core. The fatty acid and/or fatty acid salt composition becomes part of the resulting core surface following treatment of the core outer surface with the fatty acid and/or fatty acid salt composition. The fatty acid and/or fatty acid salt composition acts as a plasticizer to penetrate and soften the core surface and thereby create a gradient between the core outer surface and other core regions within the core. For example, a gradient is formed between the geometric center and the treated outer surface. The long hydrocarbon chains of the fatty acids and/or fatty acid salts increase the free volume between the polymer chains to soften the crosslinked network resulting in a lower hardness measurement.

The fatty acid and/or fatty acid salt compositions maintain plasticizer permanence within the core surface through several mechanisms. Fatty acid salts inherently have low volatility and permanence due to their ability to solidify and/or crystallize within the polymer network minimizing or eliminating migration. Although the fatty acid salts solidify and/or crystallize, they continue to reduce the hardness of the original crosslinked network. The fatty acids are highly compatible with the polymer network aiding in plasticizer permanence. Additionally, since the core formulations contain significant amounts of reactive metal oxides and/or metal salts, the fatty acids will react or coordinate with the various cation sources in the polymer matrix improving the thermal stability and permanence of the plasticizer. Furthermore, a free radical initiator can be used in conjunction with the fatty acids and/or fatty acid salts, especially when the fatty acids and/or fatty acid salts contain some unsaturation, to covalently bond the plasticizer to the polymer network further improving the plasticizer permanence.

#### DETAILED DESCRIPTION OF THE INVENTION

The present invention is directed to methods for treating golf ball cores to reduce core surface hardness, and to golf balls having reduced surface hardness. In a first embodiment, an untreated thermoset rubber golf ball core comprising an untreated outer surface having an untreated surface hardness, is treated with a surface-softening material comprising at least one fatty acid or fatty acid salt composition. The resulting treated golf ball core comprises a treated outer surface having a hardness which is less than the hardness of the untreated outer surface. Then, at least one cover layer is formed about the treated core to form the golf ball.

The thermoset rubber composition may comprise, for example, polybutadiene compositions as discussed herein. The terms thermoset rubber, cured rubber, and crosslinked rubber are used interchangeably herein, and all refer to a diene rubber composition which has undergone at least some degree of polymerization.

The step of treating typically includes but is not limited to coating, rolling, dipping, soaking, spraying, dusting, or exposing the untreated golf ball core to at least one fatty acid or fatty acid salt composition or blends/combinations thereof.

The at least one fatty acid or fatty acid salt composition may include, for example, oleic acid, palmitic acid, stearic acid, behenic acid, pelargonic acid, linoleic acid, linolenic acid, arachidonic acid, caproic acid, caprylic acid, capric acid, lauric acid, erucic acid, myristic acid, benzoic acid, phenylacetic acid, or naphthalenoic acid. The at least one fatty acid or fatty acid salt composition may further include antioxidants, sulfur-bearing compounds, zinc methacrylate, zinc dimethacrylate, softening acrylate monomers or oligomers, soft powdered thermoplastic resins, phenol-comprising antioxidants, or hydroquinones.

The untreated golf ball core may also include other compositions for modifying the properties of the core surface, such as thermoplastic elastomers and other polymers, also discussed herein.

In addition, the step of treating the untreated core with the fatty acid or fatty acid salt composition or blends/combinations of the present invention may be followed by a subsequent step of neutralizing the treated core/preform surface, either partially or fully, with a cation or other suitable source. Suitable cation sources include but are not limited to barium, lithium, sodium, zinc, bismuth, chromium, cobalt, copper, potassium, strontium, titanium, tungsten, magnesium, cesium, iron, nickel, silver, aluminum, tin and calcium.

In a further embodiment, an untreated crosslinked golf ball core comprising a thermoset rubber composition has a geometric center and an untreated outer surface, each having a hardness. The untreated crosslinked golf ball core is treated with a surface-softening material comprising at least one fatty acid or fatty acid salt composition. A golf ball core is then formed comprising a treated outer surface having a hardness less than the hardness of the untreated outer surface. The treated outer surface may further have a surface hardness less than the hardness of the geometric center of the untreated golf ball core to define a negative hardness gradient. Then, a cover layer is formed about the core to form the golf ball.

In an alternative embodiment, a preform comprising an uncured polybutadiene composition is coated with a first surface-softening material comprising at least one of a fatty acid compound or a fatty acid salt compound. Following treatment with the fatty acid and/or fatty acid salt compositions, the uncured treated golf ball core material may be compression molded at a predetermined temperature for a predetermined time, e.g. 330-360° F. for 11 minutes to form a molded core. A crosslinked golf ball core is thus formed having an outer surface having a first hardness and a geometric center having a second hardness greater than the first to define a negative hardness gradient. Then, optionally, the molded core may also be subjected to Gleber or centerless grinding. A cover layer is then formed about the core to form the golf ball.

In another embodiment, a polybutadiene composition is extruded to form a cylindrical extrudate and the extrudate is cut to form an uncured polybutadiene preform. The preform is then cold formed into a sphere, and uniformly coated with a surface-softening material comprising at least one fatty acid and/or fatty acid salt composition. In a preferred embodiment, the preform is subjected to centerless grinding prior to the treating step. The core may also be preheated to a predetermined temperature followed by treatment with the fatty acid and/or fatty acid salt composition. The coated preform is then cured to form a crosslinked core having an outer surface having a first hardness and a geometric center having a second hardness greater than the first to define a negative hardness gradient. In an alternative embodiment, the cured core is subsequently subjected to center-less grinding to form a uniformly-spherical core having increased surface roughness, an

inner cover layer is formed about the uniformly-spherical core, and an outer cover layer is formed about the inner cover layer to form the golf ball. The core may also alternatively be heated at a predetermined temperature for a predetermined time following treatment with the fatty acid/fatty acid salt composition.

In one embodiment, the thermoset rubber composition core is partially cured before the step of treating the core with the surface-softening materials of the present invention. Following treatment, the treated core is subjected to conditions, for example, heat, in order to affect additional curing or crosslinking. Additionally, the golf ball core may comprise several layers which are treated with a surface-softening material comprising at least one fatty acid or fatty acid salt composition or blends/combinations thereof.

In one embodiment, a golf ball comprises a core and a cover, wherein the core has an outer surface that is treated with at least one fatty acid such that the outer surface has a hardness ratio (R) of the hardness after treatment ( $H_2$ ) to the hardness before treatment ( $H_1$ ) of less than about 0.95.

In yet another embodiment, a golf ball comprises a core and a cover, wherein the core has a geometric center having a hardness ( $H_g$ ) and the core has an outer surface that is treated with at least one fatty acid or fatty acid salt such that the outer surface has an extrapolated hardness ( $H_E$ ) and an actual hardness ( $H_{OS}$ ) wherein  $H_E$  is derived from a five point extrapolation within three quarters of an outer core diameter and  $H_{OS}$  is measured on the curved surface of the core, and the cover has a hardness ( $H_C$ ), wherein  $H_C > H_E > H_g > H_{OS}$ .

In still another embodiment, a golf ball comprises a core and a cover, wherein the core has a geometric center having a hardness ( $H_g$ ) and the core has an outer surface that is treated with at least one fatty acid or fatty acid salt such that the outer surface has an extrapolated hardness ( $H_E$ ) and an actual hardness ( $H_{OS}$ ) wherein  $H_E$  is derived from a five point extrapolation within three quarters of an outer core diameter and  $H_{OS}$  is measured on the curved surface of the core, and the cover has a hardness ( $H_C$ ), wherein  $H_E > H_g > H_{OS} > H_C$ .

The balls of the present invention may include a single-layer (one-piece) golf ball, two-piece golf ball (core and cover) and multi-layer or multi-piece golf balls, such as one having a core of one or more layers and a cover of one or more layers surrounding the core, but are preferably formed from a core comprised of a solid center (otherwise known as an inner core) and an outer core layer, an inner cover layer and an outer cover layer. Of course, any of the core and/or the cover layers may include more than one layer. In a preferred embodiment, the core is formed of an inner core and an outer core layer where both the inner core and the outer core layer have a "soft-to-hard" hardness gradient (a "negative" hardness gradient) radially inward from each component's outer surface towards its innermost portion (i.e., the center of the inner core or the inner surface of the outer core layer), although alternative embodiments involving varying direction and combination of hardness gradient amongst core components are also envisioned (e.g., a "negative" gradient in the center coupled with a "positive" gradient in the outer core layer, or vice versa).

The center of the core may also be a liquid-filled or hollow sphere surrounded by one or more intermediate and/or cover layers, or it may include a solid or liquid center around which tensioned elastomeric material is wound. Any layers disposed around these alternative centers may exhibit the inventive core surface-softening. The cover layer may be a single layer or, for example, formed of a plurality of layers, such as an inner cover layer and an outer cover layer.

As briefly discussed above, the inventive cores may have a hardness gradient defined by hardness measurements made at the surface of the inner core (or outer core layer) and radially inward toward the center of the inner core, typically at 2-mm increments. As used herein, the terms "negative" and "positive" refer to the result of subtracting the hardness value at the innermost portion of the component being measured (e.g., the center of a solid core or an inner core in a dual core construction; the inner surface of a core layer; etc.) from the hardness value at the outer surface of the component being measured (e.g., the outer surface of a solid core; the outer surface of an inner core in a dual core; the outer surface of an outer core layer in a dual core, etc.). For example, if the outer surface of a solid core has a lower hardness value than the center (i.e., the surface is softer than the center), the hardness gradient will be deemed a "negative" gradient (a smaller number—a larger number=a negative number). It is preferred that the inventive cores have a zero or a negative hardness gradient. In one embodiment, the hardness of the treated outer surface is at least 5 Shore C less than the hardness of the untreated golfball core surface. In another embodiment, the hardness of the treated outer surface is at least 10 Shore C less than the hardness of the untreated golf ball core surface. In a preferred "negative" gradient embodiment, the core outer surface hardness is lower than the core geometric center hardness by about 0 to 30 Shore C, more preferably by about 5 to 25 Shore C lower, and at most the core outer surface hardness is about 8 to 20 Shore C lower than the core geometric center hardness.

The invention is more particularly directed to the creation of a soft "skin" on the outermost surface of the core, such as the outer surface of a single core or the outer surface of the outer core layer in a dual core construction. The "skin" is typically defined as the volume of the core that is within about 0.001 inches to about 0.200 inches of the surface, preferably about 0.003 inches to about 0.100 inches, and more preferably about 0.005 inches to about 0.060 inches. Alternatively, the volume may be within 0.008 inches to about 0.030 inches of the surface. In one embodiment, a single or multi-layer core is treated as a preform (prior to molding) by coating the surface of the preform with a surface-softening material.

The surface-softening material may be in a solid form, typically a powder, prill, gaseous or small pellet, but alternatively may be in solution form, such as a liquid, dispersion, or slurry in a solvent. Suitable solvents or carriers include, but are not limited to, water, hydrocarbon solvents, polar solvents, and plasticizers. If a liquid is used, it is preferably one that dissolves the fatty acid. Most preferably, the surface-softening material is a liquid at or near room temperature and requires no solvent.

Preferably, the layer to be treated with the surface-softening material is a core or core layer, but also in an alternative embodiment the layer is a cover or cover layer (inner or outer cover layer) comprising a diene rubber composition, preferably polybutadiene rubber.

In a preferred embodiment, the golf ball core surface or preform is coated by rolling, dipping, soaking, spraying, dusting, or otherwise exposing the core surface to at least one surface-softening material comprising at least one fatty acid or fatty acid salt composition or blends/combinations thereof.

Suitable fatty acids include but are not limited to oleic acid, palmitic acid, stearic acid, behenic acid, pelargonic acid, linoleic acid, linolenic acid, arachidonic acid, caproic acid, caprylic acid, capric acid, lauric acid, erucic acid, myristic acid, benzoic acid, phenylacetic acid, naphthalenoic acid, dimerized derivatives thereof, salts, cation, blends and combinations thereof. Certain fatty acids such as oleic acid, linoleic acid, linolenic acid, arachidonic acid are particularly

suitable because they are in liquid form at room temperature and the core can therefore be easily immersed/dipped in the neat material. Such fatty acids include, for example, oleic acid, linoleic acid, linolenic acid and arachidonic acid.

Suitable fatty acid cations include, for example, barium, lithium, sodium, zinc, bismuth, chromium, cobalt, copper, potassium, strontium, titanium, tungsten, magnesium, cesium, iron, nickel, silver, aluminum, tin and calcium.

Additional suitable surface-softening and/or cure-altering materials may be either combined directly with the fatty acid or fatty acid salt composition and blends/combinations and/or used to pretreat the preform prior to coating the perform with the fatty acid fatty acid salt compositions. Examples include, but are not limited to, antioxidants, sulfur-bearing compounds such as pentachlorothiophenol or metal salts thereof, ZDMA, softening acrylate monomers or oligomers, and soft powdered thermoplastic resins such as ethyl vinyl acetate, ethylene butyl acrylate, ethylene methyl acrylate, and very-low-modulus ionomers. Preferred additional surface softening materials include, for example, phenol-comprising antioxidants, hydroquinones, and "soft and fast" agents, such as organosulfur compounds, inorganic sulfur compounds, and thiophenols, particularly pentachlorothiophenol (PCTP) and metal salts of PCTP, such as ZnPCTP, MgPCTP, DTDS, and those disclosed in U.S. Pat. Nos. 6,458,895; 6,417,278; and 6,635,716; and U.S. Patent Application Publication Serial No. 2006/021586, the disclosures of which are incorporated herein by reference. Alternatively, thermoplastic or thermosetting powders, such as low molecular weight polyethylene, ethyl vinyl acetate, ethylene copolymers and terpolymers (i.e., NUCREL®), ethylene butyl acrylate, ethylene methyl acrylate, polyurethanes, polyureas, polyurethane-copolymers (i.e., silicone-urethanes), PEBAK®, HYTREL®, polyesters, polyamides, epoxies, silicones, and Micromorph® materials, such as those disclosed in U.S. patent application Publication Ser. Nos. 11/690,530 and 11/690,391, incorporated herein by reference.

In one particularly preferred embodiment, a polybutadiene rubber preform is coated with an antioxidant-comprising powder and then molded at 350-360° F. for 11 minutes to form a single core. The resultant core has an outer diameter of about 1.580 inches and a geometric center-point hardness of about 60 to 80 Shore C, preferably about 65 to 78 Shore C, and most preferably about 70 to 75 Shore C. At a point about 15 mm to about 20 mm from the center point of the core, the soft "skin" has a hardness of about 60 to 80 Shore C, preferably about 65 to 75 Shore C, and most preferably about 68 to 74 Shore C, resulting in an overall gradient (as measured from center to surface) of zero, and most preferably negative (i.e., about -30 to 0, more preferably about -15 to 0, most preferably about -10 to 0). The core of this example typically has an Atti compression of about 70 and a COR of about 0.800, when measured at an incoming velocity of 125 ft/s. Preferred Atti core compressions are 110 or less, preferably 100 or less, more preferably 90 or less, and most preferably 80 or less.

A second particularly preferred embodiment is a two-piece core formed from an inner core and an outer core layer. The inner core may or may not be "treated" as described herein, but preferably the outer core layer is treated to create the soft outer "skin." In one embodiment, a soft inner core is surrounded by a relatively hard outer core layer. The inner core preferably has a an outer diameter of about 1.0 inch, a center point hardness of about 55 to 60 Shore C, and an outer surface hardness of about 75 to 80 Shore C. The surface hardness of the modified "skin" of the outer core layer is about 60 to 80 Shore C, more preferably about 65 to 75 Shore C, and most preferably about 68 to 74 Shore C. A preferred overall gradi-

ent is negative to zero, most preferably negative (i.e., about -30 to 0, more preferably about -20 to -3, and most preferably about -15 to -5).

The core formulations used in the invention are preferably based upon high-cis polybutadiene rubber that is cobalt-, nickel-, lithium-, or neodymium-catalyzed, most preferably Co- or Nd-catalyzed, having a Mooney viscosity of about 25 to about 125, more preferably about 30 to about 100, and most preferably about 40 to about 60. Lesser amounts of non-polybutadiene rubber, such as styrene butadiene rubber, trans-polyisoprene, natural rubber, butyl rubber, ethylene propylene rubber, ethylene propylene diene monomer rubber, low-cis polybutadiene rubber, or trans polybutadiene rubber, may also be blended with the polybutadiene rubber. A coagent, such as zinc diacrylate or zinc dimethacrylate, is typically present at a level of about 0 pph to about 60 pph, more preferably about 10 pph to about 55 pph, and most preferably about 15 pph to about 40 pph. A peroxide or peroxide blend is also typically present at about 0.1 pph to about 5.0 pph, more preferably about 0.5 pph to about 3.0 pph. Zinc oxide may also be present at about 2 pph to about 50 pph and the antioxidant is preferably present at about 0 pph to about 5.0 pph, preferably about 0.5 pph to about 3.0 pph. Elemental sulfur may also be present in the amount of about 0.05 to 2 pph, preferably about 0.1 to 0.5 pph.

Other embodiments include any number of core layers and gradient combinations wherein at least one layer of the core has a surface that is "treated" as described herein.

Scrap automotive tire regrind (in fine powder form) is also sufficient for creating the inventive soft outer "skin," as well as other powdered rubbers that are uncrosslinked or partially crosslinked and therefore able to react with the polybutadiene. Fully crosslinked powdered rubber may also still have enough affinity for the polybutadiene substrate to adhere (even react minimally) enough to form a good bond.

The inner and outer core formulations may comprise a diene rubber, a cure initiator, and a coagent. Suitable diene rubbers include, for example, those disclosed in U.S. patent application Ser. No. 11/561,923 ('923 application), incorporated herein by reference. Suitable cure initiators include for example, peroxide or sulfur. The coagent may comprise ZDA, ZDMA, TMPTA, HVA-2 or any of those identified in the '923 application. Optionally, the formulations may also include one or more of a zinc oxide, zinc stearate or stearic acid, antioxidant, or soft to fast agent such as PCTP or ZnPCTP. Either the inner or outer core, more preferably the outer core, may further comprise from about 1 to 100 phr of a stiffening or toughening thermoplastic polymer such as an ionomer, an acid co- or ter-polymer, polyamide, polyester or any as disclosed in U.S. Pat. No. 6,120,390 or 6,284,840, incorporated herein by reference. Preferably, the inner and outer core layers comprise a high cis-neodymium catalyzed polybutadiene such as Neodene 40 or CB-23, or a cobalt or nickel or lithium catalyzed PBR such as BR-1220 or BR-221. A trans PIP, for example balata TP-301, or trans BR may be used to add stiffness to the cores and/or improve cold forming properties, particularly for ease of molding a half-shell for the outer core formation.

Other potential surface-softening or cure-altering agents include, but are not limited to, sulfated fats, sodium salts of alkylated aromatic sulfonic acids, substituted benzoid alkyl sulfonic acids, monoaryl and alkyl ethers of diethylene glycol and dipropylene glycol, ammonium salts of alkyl phosphates, sodium alkyl sulfates and monosodium salt of sulfated methyl oleate and sodium salts of carboxylated electrolytes. Other suitable materials include dithiocarbamates, such as zinc dimethyl dithiocarbamate, zinc diethyl dithiocarbamate, zinc

13

di-n-butyl dithiocarbamate, zinc diamyl dithiocarbamate, tellurium diethyl dithiocarbamate, selenium dimethyl dithiocarbamate, selenium diethyl dithiocarbamate, lead diamyl dithiocarbamate, bismuth dimethyl dithiocarbamate, cadmium diethyl dithiocarbamate, and mixtures thereof.

The method for making the golf ball of the invention includes a variety of steps and options. Typically, a Banbury-type mixer or the like is used to mix the polybutadiene rubber composition. The rubber composition is extruded as an extrudate and cut to a predetermined shape, such as a cylinder, typically called a "preform". The preform comprising the uncured polybutadiene composition is then prepared for coating with at least one of the surface-softening (inhibiting) materials, liquids, or solvents described above. Other surface-softening and/or cure-altering materials may be added for coating, comprising antioxidants, sulfur-bearing compounds, zinc methacrylate, zinc dimethacrylate, softening acrylate monomers or oligomers, soft powdered thermoplastic resins, phenol-comprising antioxidants, or hydroquinones, most preferably an antioxidant.

In one embodiment, more than one surface-softening material is used, in succession. In this embodiment, a preferred combination includes a first surface-softening material in combination with a cure-altering material such as an antioxidant and a second cure-altering material such as a different antioxidant or a peroxide. A compatibilizer and/or tie layer may be incorporated as well. Additionally, a two-stage dip or roll (in the cure-altering material) may be used to sequentially also provide a first and second antioxidant or an antioxidant and a peroxide in addition to providing the fatty acid and/or fatty acid salt composition.

Optionally, prior to coating the preform, the uncured preform may be shaped or cold-formed into a rough sphere. The coating may be performed in a variety of manners including, but not limited to, rolling, spraying, dipping, or dusting or otherwise exposing. The coating may be uniform or varied, but is preferably uniform.

The uncured, coated preform may optionally be heated to a predetermined temperature for a predetermined time, the temperature being substantially below the predetermined cure temperature, so that the cure-altering material may diffuse, penetrate, migrate, or otherwise work its way into the preform or, alternatively, any solvent may evaporate or the preform may dry (if the coating was in liquid form). Where two surface-softening materials are employed in a coating, or in the case where a surface-softening material is used in combination with a cure-altering material as the coating material, the predetermined time may also be set in order to allow any reaction that may occur to come to completion.

The uncured coated preform is then cured or molded at a predetermined temperature and time to form a crosslinked golf ball core. As described in detail above, the core has an outer surface having a first hardness and a geometric center having a second hardness greater than the first to define a "negative" hardness gradient. Any one of a number of cover layers may be formed around the "negative" gradient core including, but not limited to, an outer core layer, an inner cover layer, and an outer cover layer.

The cured core is then typically subjected to centerless-grinding so that the core is uniformly spherical and has a surface that is roughened and textured to be better suited for adhesion with subsequent layers. Prior to or after the centerless grinding, the core may be treated with plasma discharge, corona discharge, silanes, or chlorination, for example, to aid in its adhesion properties.

In a preferred embodiment, a thermoset rubber core is soaked in a liquid fatty acid composition including, for

14

example, oleic acid. Following the soaking step, the core is removed from the surface-softening composition and wiped dry in order to remove any excess oleic acid. A cover layer is then molded over the treated core. Preferably, the surface 5 hardness is reduced from about 85 Shore C to about 83 Shore C or less, and more preferably, to about 80 Shore C or less. In one embodiment, a negative gradient may be created if the Shore C surface hardness after treatment is about 60 Shore C or less and the center hardness is about 62 Shore C. The 10 degree of resulting core surface softness is directly related to the duration of core surface exposure to the surface-softening composition so that a particular resulting core surface hardness may be achieved by varying the duration of exposure.

Alternatively, the fatty acid may comprise a heated molten 15 form of magnesium oleate. Additionally, the core may be exposed i.e., dipped or soaked, in a solvent solution of stearic acid and zinc oxide in tetrahydrofuran (THF).

In one embodiment, the untreated thermoset rubber golf 20 ball core has an outer diameter of 1.400-1.640 inches, and more preferably 1.50-1.62 inches, and most preferably 1.55-1.60 inches. Additionally, the thermoset rubber golf ball core has a compression of about 30-120, and more preferably 40-110, and most preferably 60-105. Further, the untreated 25 core has a Shore C surface hardness of about 50-95, or more preferably about 60-93 Shore C, and most preferably in the range of about 75-89 Shore C. The core is dipped in oleic acid at a temperature of about 40-350° F. for a time of about 1 second to about 24 hours. More preferably, the temperature 30 and duration is 50-150° F. for about 1 minute to about 12 hours. Most preferably, the temperature and duration are about 60-110° F. for about 5 minutes, to about 6 hours, respectively. The resulting treated core has a surface hardness of about 1 to 50 Shore C lower than the surface hardness of the 35 untreated core, or more preferably about 5 to 25 Shore C lower, and most preferably about 10 to 20 Shore C lower.

One embodiment includes the steps of extruding a polybutadiene composition to form a cylindrical extrudate; cutting the extrudate to form an uncured polybutadiene preform; 40 uniformly coating the preform with a cure-altering material comprising a first antioxidant; curing the coated preform to form a crosslinked core having an outer surface having a first hardness and a geometric center having a second hardness greater than the first to define a negative hardness gradient; centerless-grinding the cured core to form a uniformly-spherical core having increased surface roughness; forming an inner cover layer about the uniformly-spherical core; and forming an outer cover layer about the inner cover layer to form the golf ball.

In yet another embodiment, a thermoset rubber or at least 45 partially cured diene rubber composition is ground, pulverized or otherwise converted into the form of a particle having a regular or irregular shape and a particle size of from about 1 nm to about 2 mm in diameter (or maximum cross sectional length). The ground thermoset rubber may be formed by grinding a thermoset golf ball core to a sieve size of about 10-40 mesh. Such a ground golf ball core is commonly referred to as golf ball core regrind. The ground thermoset rubber is then treated with a fatty acid or fatty acid salt 50 comprising composition to soften at least the surface of the ground particle. The treated ground thermoset rubber particles are then admixed with an uncured diene rubber composition followed by the steps needed to form a golf ball core, ie extrusion, forming a preform, crosslinking into a spherical core, etc. The addition of the treated ground thermoset rubber 55 to the diene rubber composition is meant to soften and perhaps enhance the feel of the molded core comprising the

treated ground rubber, and lower core compression while having little adverse effect on core speed.

Preferably, the core layers (inner core or outer core layer) is made from a composition including at least one thermoset base rubber, such as a polybutadiene rubber, cured with at least one peroxide and at least one reactive co-agent, which can be a metal salt of an unsaturated carboxylic acid, such as acrylic acid or methacrylic acid, a non-metallic coagent, or mixtures thereof. Preferably, a suitable antioxidant is included in the composition. An optional soft and fast agent (and sometimes a cis-to-trans catalyst), such as an organosulfur or metal-containing organosulfur compound, can also be included in the core formulation.

Other ingredients that are known to those skilled in the art may be used, and are understood to include, but not be limited to, density-adjusting fillers, process aides, plasticizers, blowing or foaming agents, sulfur accelerators, and/or non-peroxide radical sources.

The base thermoset rubber, which can be blended with other rubbers and polymers, typically includes a natural or synthetic rubber. A preferred base rubber is 1,4-polybutadiene having a cis structure of at least 40%, preferably greater than 80%, and more preferably greater than 90%.

Examples of desirable polybutadiene rubbers include BUNA® CB22 and BUNA® CB23, commercially available from LANXESS Corporation; UBEPOL® 360L and UBEPOL® 150L and UBEPOL-BR rubbers, commercially available from UBE Industries, Ltd. of Tokyo, Japan; KINEX® 7245 and KINEX® 7265, commercially available from Goodyear of Akron, Ohio; Shell BR-1220, commercially available from Dow chemical Company, Europrene®NEOCIS® BR 40 and BR 60, commercially available from Polimeri Europa; and BR 01, BR 730, BR 735, BR 11, and BR 51, commercially available from Japan Synthetic Rubber Co., Ltd; PETROFLEX® BRNd-40; and KARBOCHEM® ND40, ND45, and ND60, commercially available from Karbochem.

The base rubber may also comprise high or medium Mooney viscosity rubber, or blends thereof. A "Mooney" unit is a unit used to measure the plasticity of raw or unvulcanized rubber. The plasticity in a "Mooney" unit is equal to the torque, measured on an arbitrary scale, on a disk in a vessel that contains rubber at a temperature of 100° C. and rotates at two revolutions per minute. The measurement of Mooney viscosity is defined according to ASTM D-1646.

The Mooney viscosity range is preferably greater than about 40, more preferably in the range from about 40 to about 80 and more preferably in the range from about 40 to about 60. Polybutadiene rubber with higher Mooney viscosity may also be used, so long as the viscosity of the polybutadiene does not reach a level where the high viscosity polybutadiene clogs or otherwise adversely interferes with the manufacturing machinery. It is contemplated that polybutadiene with viscosity less than 65 Mooney can be used with the present invention.

In one embodiment of the present invention, golf ball cores made with mid- to high-Mooney viscosity polybutadiene material exhibit increased resiliency (and, therefore, distance) without increasing the hardness of the ball. Such cores are soft, i.e., compression less than about 60 and more specifically in the range of about 50-55. Cores with compression in the range of from about 30 about 50 are also within the range of this preferred embodiment.

Commercial sources of suitable mid- to high-Mooney viscosity polybutadiene include Bayer AG CB23 (Nd-catalyzed), which has a Mooney viscosity of around 50 and is a highly linear polybutadiene, and Shell 1220 (Co-catalyzed).

If desired, the polybutadiene can also be mixed with other elastomers known in the art, such as other polybutadiene rubbers, natural rubber, styrene butadiene rubber, and/or isoprene rubber in order to further modify the properties of the core. When a mixture of elastomers is used, the amounts of other constituents in the core composition are typically based on 100 parts by weight of the total elastomer mixture.

In one preferred embodiment, the base rubber comprises a Nd-catalyzed polybutadiene, a rare earth-catalyzed polybutadiene rubber, or blends thereof. If desired, the polybutadiene can also be mixed with other elastomers known in the art such as natural rubber, polyisoprene rubber and/or styrene-butadiene rubber in order to modify the properties of the core. Other suitable base rubbers include thermosetting materials such as, ethylene propylene diene monomer rubber, ethylene propylene rubber, butyl rubber, halobutyl rubber, hydrogenated nitrile butadiene rubber, nitrile rubber, and silicone rubber.

Thermoplastic elastomers (TPE) may also be used to modify the properties of the core layers, or the uncured core layer stock by blending with the base thermoset rubber. These TPEs include natural or synthetic balata, or high trans-polyisoprene, high trans-polybutadiene, or any styrenic block copolymer, such as styrene ethylene butadiene styrene, styrene-isoprene-styrene, etc., a metallocene or other single-site catalyzed polyolefin such as ethylene-octene, or ethylene-butene, or thermoplastic polyurethanes (TPU), including copolymers, e.g. with silicone. Other suitable TPEs for blending with the thermoset rubbers of the present invention include PEBAK®, which is believed to comprise polyether amide copolymers, HYTREL®, which is believed to comprise polyether ester copolymers, thermoplastic urethane, and KRATON®, which is believed to comprise styrenic block copolymers elastomers. Any of the TPEs or TPUs above may also contain functionality suitable for grafting, including maleic acid or maleic anhydride.

Suitable peroxide initiating agents include dicumyl peroxide; 2,5-dimethyl-2,5-di(t-butylperoxy)hexane; 2,5-dimethyl-2,5-di(t-butylperoxy)hexyne; 2,5-dimethyl-2,5-di(benzoylperoxy)hexane; 2,2-bis(t-butylperoxy)-di-isopropylbenzene; 1,1-bis(t-butylperoxy)-3,3,5-trimethyl cyclohexane; n-butyl 4,4-bis(t-butylperoxy)valerate; t-butyl perbenzoate; benzoyl peroxide; n-butyl 4,4'-bis(butylperoxy)valerate; di-t-butyl peroxide; or 2,5-di-(t-butylperoxy)-2,5-dimethyl hexane, lauryl peroxide, t-butyl hydroperoxide,  $\alpha$ - $\alpha$  bis(t-butylperoxy)diisopropylbenzene, di(2-t-butylperoxyisopropyl)benzene, di-t-amyl peroxide, di-t-butyl peroxide. Preferably, the rubber composition includes from about 0.25 to about 5.0 parts by weight peroxide per 100 parts by weight rubber (phr), more preferably 0.5 phr to 3 phr, most preferably 0.5 phr to 1.5 phr. In a most preferred embodiment, the peroxide is present in an amount of about 0.8 phr. These ranges of peroxide are given assuming the peroxide is 100% active, without accounting for any carrier that might be present.

Because many commercially available peroxides are sold along with a carrier compound, the actual amount of active peroxide present must be calculated. Commercially-available peroxide initiating agents include DICUP™ family of dicumyl peroxides (including DICUP™ R, DICUP™ 40C and DICUP™ 40KE) available from Crompton (Geo Specialty Chemicals). Similar initiating agents are available from AkroChem, Lanxess, Flexsys/Harwick and R.T. Vanderbilt. Another commercially-available and preferred initiating agent is TRIGONOX™ 265-50B from Akzo Nobel, which is a mixture of 1,1-di(t-butylperoxy)-3,3,5-trimethylcyclohexane and di(2-t-butylperoxyisopropyl)benzene. TRIGONOX™ peroxides are generally sold on a carrier compound.

Suitable reactive co-agents include, but are not limited to, metal salts of diacrylates, dimethacrylates, and monomethacrylates suitable for use in this invention include those wherein the metal is zinc, magnesium, calcium, barium, tin, aluminum, lithium, sodium, potassium, iron, zirconium, and bismuth. Zinc diacrylate (ZDA) is preferred, but the present invention is not limited thereto. ZDA provides golf balls with a high initial velocity. The ZDA can be of various grades of purity. For the purposes of this invention, the lower the quantity of zinc stearate present in the ZDA the higher the ZDA purity. ZDA containing less than about 10% zinc stearate is preferable. More preferable is ZDA containing about 4-8% zinc stearate. Suitable, commercially available zinc diacrylates include those from Sartomer Co. The preferred concentrations of ZDA that can be used are about 10 phr to about 40 phr, more preferably 20 phr to about 35 phr, most preferably 25 phr to about 35 phr. In a particularly preferred embodiment, the reactive co-agent is present in an amount of about 29 phr to about 31 phr.

Additional preferred co-agents that may be used alone or in combination with those mentioned above include, but are not limited to, trimethylolpropane trimethacrylate, trimethylolpropane triacrylate, and the like. It is understood by those skilled in the art, that in the case where these co-agents may be liquids at room temperature, it may be advantageous to disperse these compounds on a suitable carrier to promote ease of incorporation in the rubber mixture.

Antioxidants are compounds that inhibit or prevent the oxidative breakdown of elastomers, and/or inhibit or prevent reactions that are promoted by oxygen radicals. Some exemplary antioxidants that may be used in the present invention include, but are not limited to, quinoline type antioxidants, amine type antioxidants, and phenolic type antioxidants. A preferred antioxidant is 2,2'-methylene-bis-(4-methyl-6-t-butylphenol) available as VANOX® MBPC from R.T. Vanderbilt. Other polyphenolic antioxidants include VANOX® T, VANOX® L, VANOX® SKT, VANOX® SWP, VANOX® 13 and VANOX® 1290.

The antioxidant is typically present in an amount of about 0.1 phr to about 5 phr, preferably from about 0.1 phr to about 2 phr, more preferably about 0.1 phr to about 1 phr. In a particularly preferred embodiment, the antioxidant is present in an amount of about 0.4 phr. In an alternative embodiment, the antioxidant should be present in an amount to ensure that the hardness gradient of the inventive cores is negative. Preferably, about 0.2 phr to about 1 phr antioxidant is added to the core layer (inner core or outer core layer) formulation, more preferably, about 0.3 to about 0.8 phr, and most preferably 0.4 to about 0.7 phr. Preferably, about 0.25 phr to about 1.5 phr of peroxide as calculated at 100% active can be added to the core formulation, more preferably about 0.5 phr to about 1.2 phr, and most preferably about 0.7 phr to about 1.0 phr. The ZDA amount can be varied to suit the desired compression, spin and feel of the resulting golf ball. The cure regime can have a temperature range between from about 290° F. to about 400° F., more preferably about 325° F. to about 360° F., and the stock is held at that temperature for at least about 10 minutes to about 30 minutes.

The thermoset rubber composition of the present invention may also include an optional soft and fast agent. As used herein, "soft and fast agent" means any compound or a blend thereof that is capable of making a core 1) be softer (lower compression) at constant COR or 2) have a higher COR at equal compression, or any combination thereof, when compared to a core equivalently prepared without a soft and fast agent. Preferably, the composition of the present invention contains from about 0.05 phr to about 10.0 phr soft and fast

agent. In one embodiment, the soft and fast agent is present in an amount of about 0.05 phr to about 3.0 phr, preferably about 0.05 phr to about 2.0 phr, more preferably about 0.05 phr to about 1.0 phr. In another embodiment, the soft and fast agent is present in an amount of about 2.0 phr to about 5.0 phr, preferably about 2.35 phr to about 4.0 phr, and more preferably about 2.35 phr to about 3.0 phr. In an alternative high concentration embodiment, the soft and fast agent is present in an amount of about 5.0 phr to about 10.0 phr, more preferably about 6.0 phr to about 9.0 phr, most preferably about 7.0 phr to about 8.0 phr. In a most preferred embodiment, the soft and fast agent is present in an amount of about 2.6 phr.

Suitable soft and fast agents include, but are not limited to, organosulfur or metal-containing organosulfur compounds, an organic sulfur compound, including mono, di, and polysulfides, a thiol, or mercapto compound, an inorganic sulfide compound, a Group VIA compound, or mixtures thereof. The soft and fast agent component may also be a blend of an organosulfur compound and an inorganic sulfide compound.

Suitable soft and fast agents of the present invention include, but are not limited to those having the following general formula:



where R<sub>1</sub>-R<sub>5</sub> can be C<sub>1</sub>-C<sub>8</sub> alkyl groups; halogen groups; thiol groups (—SH), carboxylated groups; sulfonated groups; and hydrogen; in any order; and also pentafluorothiophenol; 2-fluorothiophenol; 3-fluorothiophenol; 4-fluorothiophenol; 2,3-fluorothiophenol; 2,4-fluorothiophenol; 3,4-fluorothiophenol; 3,5-fluorothiophenol; 2,3,4,5-tetrafluorothiophenol; 2,3,5,6-tetrafluorothiophenol; 4-chlorotetrafluorothiophenol; pentachlorothiophenol; 2-chlorothiophenol; 3-chlorothiophenol; 4-chlorothiophenol; 2,3-chlorothiophenol; 2,4-chlorothiophenol; 3,4-chlorothiophenol; 3,5-chlorothiophenol; 2,3,4-chlorothiophenol; 3,4,5-chlorothiophenol; 2,3,4,5-tetrachlorothiophenol; 2,3,5,6-tetrachlorothiophenol; pentabromothiophenol; 2-bromothiophenol; 3-bromothiophenol; 4-bromothiophenol; 2,3-bromothiophenol; 2,4-bromothiophenol; 3,4-bromothiophenol; 3,5-bromothiophenol; 2,3,4-bromothiophenol; 3,4,5-bromothiophenol; 2,3,4,5-tetrabromothiophenol; 2,3,5,6-tetrabromothiophenol; pentaiodothiophenol; 2-iodothiophenol; 3-iodothiophenol; 4-iodothiophenol; 2,3-iodothiophenol; 2,4-iodothiophenol; 3,4-iodothiophenol; 3,5-iodothiophenol; 2,3,4-iodothiophenol; 3,4,5-iodothiophenol; 2,3,4,5-tetraiodothiophenol; 2,3,5,6-tetraiodothiophenol; and their zinc salts. Preferably, the halogenated thiophenol compound is pentachlorothiophenol, which is commercially available in neat form or under the tradename STRUKTOL®, a clay-based carrier containing the sulfur compound pentachlorothiophenol loaded at 45 percent. STRUKTOL® is commercially available from Struktol Company of America of Stow, Ohio. PCTP is commercially available in neat form from eChinachem of San Francisco, Calif. and in the salt form from eChinachem of San Francisco, Calif. Most preferably, the halogenated thiophenol compound is the zinc salt of pen-

19

tachlorothiophenol, which is commercially available from eChinachem of San Francisco, Calif.

Other suitable soft and fast agents include, but are not limited to, hydroquinones, benzoquinones, quinhydrone, catechols, and resorcinols.

Suitable hydroquinone compounds include compounds represented by the following formula, and hydrates thereof:



wherein each R<sub>1</sub>, R<sub>2</sub>, R<sub>3</sub>, and R<sub>4</sub> are hydrogen; halogen; alkyl; carboxyl; metal salts thereof, and esters thereof; acetate and esters thereof; formyl; acyl; acetyl; halogenated carbonyl; sulfo and esters thereof; halogenated sulfonyl; sulfino; alkylsulfinyl; carbamoyl; halogenated alkyl; cyano; alkoxy; hydroxy and metal salts thereof; amino; nitro; aryl; aryloxy; arylalkyl; nitroso; acetamido; or vinyl.

Other suitable hydroquinone compounds include, but are not limited to, hydroquinone; tetrachlorohydroquinone; 2-chlorohydroquinone; 2-bromohydroquinone; 2,5-dichlorohydroquinone; 2,5-dibromohydroquinone; tetrabromohydroquinone; 2-methylhydroquinone; 2-t-butylhydroquinone; 2,5-di-t-amylhydroquinone; and 2-(2-chlorophenyl)hydroquinone hydrate.

More suitable hydroquinone compounds include compounds represented by the following formula, and hydrates thereof:



wherein each R<sub>1</sub>, R<sub>2</sub>, R<sub>3</sub>, and R<sub>4</sub> are a metal salt of a carboxyl; acetate and esters thereof; hydroxy; a metal salt of a hydroxy; amino; nitro; aryl; aryloxy; arylalkyl; nitroso; acetamido; or vinyl.

Suitable benzoquinone compounds include compounds represented by the following formula, and hydrates thereof:



wherein each R<sub>1</sub>, R<sub>2</sub>, R<sub>3</sub>, and R<sub>4</sub> are hydrogen; halogen; alkyl; carboxyl; metal salts thereof, and esters thereof; acetate and esters thereof; formyl; acyl; acetyl; halogenated carbonyl; sulfo and esters thereof; halogenated sulfonyl; sulfino; alkylsulfinyl; carbamoyl; halogenated alkyl; cyano; alkoxy; hydroxy and metal salts thereof; amino; nitro; aryl; aryloxy; arylalkyl; nitroso; acetamido; or vinyl.

20

hydroxy and metal salts thereof; amino; nitro; aryl; aryloxy; arylalkyl; nitroso; acetamido; or vinyl.

Other suitable benzoquinone compounds include one or more compounds represented by the following formula, and hydrates thereof:



wherein each R<sub>1</sub>, R<sub>2</sub>, R<sub>3</sub>, and R<sub>4</sub> are a metal salt of a carboxyl; acetate and esters thereof; hydroxy; a metal salt of a hydroxy; amino; nitro; aryl; aryloxy; arylalkyl; nitroso; acetamido; or vinyl.

Suitable quinhydrone include one or more compounds represented by the following formula, and hydrates thereof:



wherein each R<sub>1</sub>, R<sub>7</sub>, R<sub>3</sub>, R<sub>4</sub>, R<sub>5</sub>, R<sub>6</sub>, R<sub>7</sub>, and R<sub>8</sub> are hydrogen; halogen; alkyl; carboxyl; metal salts thereof, and esters thereof; acetate and esters thereof; formyl; acyl; acetyl; halogenated carbonyl; sulfo and esters thereof; halogenated sulfonyl; sulfino; alkylsulfinyl; carbamoyl; halogenated alkyl; cyano; alkoxy; hydroxy and metal salts thereof; amino; nitro; aryl; aryloxy; arylalkyl; nitroso; acetamido; or vinyl.

Other suitable quinhydrone include those having the above formula, wherein each R<sub>1</sub>, R<sub>2</sub>, R<sub>3</sub>, R<sub>4</sub>, R<sub>5</sub>, R<sub>6</sub>, R<sub>7</sub>, and R<sub>8</sub> are a metal salt of a carboxyl; acetate and esters thereof; hydroxy; a metal salt of a hydroxy; amino; nitro; aryl; aryloxy; arylalkyl; nitroso; acetamido; or vinyl. Suitable catechols include one or more compounds represented by the following formula, and hydrates thereof:



wherein each R<sub>1</sub>, R<sub>2</sub>, R<sub>3</sub>, and R<sub>4</sub> are hydrogen; halogen; alkyl; carboxyl; metal salts thereof, and esters thereof; acetate and esters thereof; formyl; acyl; acetyl; halogenated carbonyl; sulfo and esters thereof; halogenated sulfonyl; sulfino; alkylsulfinyl; carbamoyl; halogenated alkyl; cyano; alkoxy; hydroxy and metal salts thereof; amino; nitro; aryl; aryloxy; arylalkyl; nitroso; acetamido; or vinyl.

## 21

Suitable resorcinols include one or more compounds represented by the following formula, and hydrates thereof:



wherein each R<sub>1</sub>, R<sub>2</sub>, R<sub>3</sub>, and R<sub>4</sub> are hydrogen; halogen; alkyl; carboxyl; metal salts thereof, and esters thereof; acetate and esters thereof; formyl; acyl; acetyl; halogenated carbonyl; sulfo and esters thereof; halogenated sulfonyl; sulfino; alkyl-sulfinyl; carbamoyl; halogenated alkyl; cyano; alkoxy; hydroxy and metal salts thereof; amino; nitro; aryl; aryloxy; arylalkyl; nitroso; acetamido; or vinyl.

Fillers may also be added to the thermoset rubber composition of the core to adjust the density of the composition, up or down. Typically, fillers include materials such as tungsten, zinc oxide, barium sulfate, silica, calcium carbonate, zinc carbonate, metals, metal oxides and salts, regrind (recycled core material typically ground to about 30 mesh particle), high-Mooney-viscosity rubber regrind, trans-regrind core material (recycled core material containing high trans-isomer of polybutadiene), and the like. When trans-regrind is present, the amount of trans-isomer is preferably between about 10% and about 60%. In a preferred embodiment of the invention, the core comprises polybutadiene having a cis-isomer content of greater than about 95% and trans-regrind core material (already vulcanized) as a filler. Any particle size trans-regrind core material is sufficient, but is preferably less than about 125  $\mu\text{m}$ .

Fillers added to one or more portions of the golf ball typically include processing aids or compounds to affect rheological and mixing properties, density-modifying fillers, tear strength, or reinforcement fillers, and the like. The fillers are

## 22

generally inorganic, and suitable fillers include numerous metals or metal oxides, such as zinc oxide and tin oxide, as well as barium sulfate, zinc sulfate, calcium carbonate, barium carbonate, clay, tungsten, tungsten carbide, an array of silicas, and mixtures thereof. Fillers may also include various foaming agents or blowing agents which may be readily selected by one of ordinary skill in the art. Fillers may include polymeric, ceramic, metal, and glass microspheres may be solid or hollow, and filled or unfilled. Fillers are typically also added to one or more portions of the golf ball to modify the density thereof to conform to uniform golf ball standards. Fillers may also be used to modify the weight of the center or at least one additional layer for specialty balls, e.g., a lower weight ball is preferred for a player having a low swing speed.

Materials such as tungsten, zinc oxide, barium sulfate, silica, calcium carbonate, zinc carbonate, metals, metal oxides and salts, and regrind (recycled core material typically ground to about 30 mesh particle) are also suitable fillers.

The polybutadiene and/or any other base rubber or elastomer system may also be foamed, or filled with hollow microspheres or with expandable microspheres which expand at a set temperature during the curing process to any low specific gravity level. Other ingredients such as sulfur accelerators, e.g., tetra methylthiuram di, tri, or tetrasulfide, and/or metal-containing organosulfur components may also be used according to the invention. Suitable metal-containing organosulfur accelerators include, but are not limited to, cadmium, copper, lead, and tellurium analogs of diethyldithiocarbamate, diamylidithiocarbamate, and dimethyldithiocarbamate, or mixtures thereof. Other ingredients such as processing aids e.g., fatty acids and/or their metal salts, processing oils, dyes and pigments, as well as other additives known to one skilled in the art may also be used in the present invention in amounts sufficient to achieve the purpose for which they are typically used.

A number of cores were formed based on the formulation and cure cycle described in TABLE 1 below and core hardness values are reported in TABLE 2 below:

TABLE 1

|                             | Ex 1  | Ex 2  | Ex 3  | Comp Ex 1 | Comp Ex 2 | Comp Ex 3 |
|-----------------------------|-------|-------|-------|-----------|-----------|-----------|
| Formulation (phr)           |       |       |       |           |           |           |
| SR-526*                     | 34.0  | 34.0  | 31.2  | 29.0      | 29.0      | 29.0      |
| ZnO                         | 5     | 5     | 5     | 5         | 5         | 5         |
| BaSO <sub>4</sub>           | 11.2  | 11.2  | 16.1  | 13.8      | 13.8      | 13.8      |
| Vanox MBPC*                 | 0.40  | 0.40  | 0.40  | —         | 0.50      | —         |
| Trigonox-265-50B**          | 1.4   | 1.4   | 1.6   | —         | —         | 0.8       |
| Perkadox BC-FF***           | —     | —     | —     | 1.0       | 1.6       | —         |
| polybutadiene               | 100   | 100   | 100   | 100       | 100       | 100       |
| ZnPCTP                      | 2.35  | 2.35  | 2.60  | 2.35      | 2.35      | 2.35      |
| regrind                     | —     | —     | 17    | 17        | —         | —         |
| antioxidant/initiator ratio | 0.57  | 0.57  | 0.50  | —         | 0.31      | —         |
| Cure Temp. (° F.)           | 305   | 315   | 320   | 350       | 335       | 335       |
| Cure Time (min)             | 14    | 11    | 16    | 11        | 11        | 11        |
| Properties                  |       |       |       |           |           |           |
| diameter (in)               | 1.530 | 1.530 | 1.530 | 1.530     | 1.530     | 1.530     |
| compression                 | 69    | 63    | 70    | 69        | 47        | —         |
| COR @ 125 ft/s              | 0.808 | 0.806 | 0.804 | 0.804     | —         | —         |

\*Vanox MBPC: 2,2'-methylene-bis-(4-methyl-6-t-butylphenol) available from R. T. Vanderbilt Company Inc.;

\*\*Trigonox 265-50B: a mixture of 1,1-di(t-butylperoxy)-3,3,5-trimethylcyclohexane and di(2-t-butylperoxyisopropyl)benzene 50% active on an inert carrier available from Akzo Nobel;

\*\*\*Perkadox BC-FF: Dicumyl peroxide (99%-100% active) available from Akzo Nobel; and

\*SR-526: ZDA available from Sartomer

TABLE 2

| Distance from Center | Shore C Hardness |      |      |           |           |           |
|----------------------|------------------|------|------|-----------|-----------|-----------|
|                      | Ex 1             | Ex 2 | Ex 3 | Comp Ex 1 | Comp Ex 2 | Comp Ex 3 |
| Center               | 73               | 70   | 71   | 61        | 52        | 61        |
| 2                    | 74               | 71   | 72   | 67        | 57        | 62        |
| 4                    | 74               | 72   | 73   | 70        | 62        | 65        |
| 6                    | 75               | 73   | 73   | 72        | 64        | 67        |
| 8                    | 75               | 73   | 73   | 73        | 64        | 69        |
| 10                   | 75               | 73   | 74   | 73        | 64        | 71        |
| 12                   | 74               | 74   | 73   | 72        | 66        | 72        |
| 14                   | 74               | 74   | 72   | 73        | 70        | 73        |
| 16                   | 70               | 71   | 70   | 77        | 71        | 73        |
| 18                   | 60               | 60   | 63   | 80        | 72        | 73        |
| Surface              | 63               | 70   | 66   | 85        | 73        | 74        |
| Surface - Center     | -10              | 0    | -5   | 24        | 21        | 13        |

The surface hardness of a core is obtained from the average of a number of measurements taken from opposing hemispheres of a core, taking care to avoid making measurements on the parting line of the core or on surface defects, such as holes or protrusions. Hardness measurements are made pursuant to ASTM D-2240 "Indentation Hardness of Rubber and Plastic by Means of a Durometer." Because of the curved surface of a core, care must be taken to insure that the core is centered under the durometer indentor before a surface hardness reading is obtained. A calibrated, digital durometer, capable of reading to 0.1 hardness units is used for all hardness measurements and is set to take hardness readings at 1 second after the maximum reading is obtained. The digital durometer must be attached to, and its foot made parallel to, the base of an automatic stand, such that the weight on the durometer and attack rate conform to ASTM D-2240.

To prepare a core for hardness gradient measurements, the core is gently pressed into a hemispherical holder having an internal diameter approximately slightly smaller than the diameter of the core, such that the core is held in place in the hemispherical portion of the holder while concurrently leaving the geometric central plane of the core exposed. The core is secured in the holder by friction, such that it will not move during the cutting and grinding steps, but the friction is not so excessive that distortion of the natural shape of the core would result. The core is secured such that the parting line of the core is roughly parallel to the top of the holder. The diameter of the core is measured 90 degrees to this orientation prior to securing. A measurement is also made from the bottom of the holder to the top of the core to provide a reference point for future calculations. A rough cut, made slightly above the exposed geometric center of the core using a band saw or other appropriate cutting tool, making sure that the core does not move in the holder during this step. The remainder of the core, still in the holder, is secured to the base plate of a surface grinding machine. The exposed 'rough' core surface is ground to a smooth, flat surface, revealing the geometric center of the core, which can be verified by measuring the height of the bottom of the holder to the exposed surface of the core, making sure that exactly half of the original height of the core, as measured above, has been removed to within  $\pm 0.004$  inches.

Leaving the core in the holder, the center of the core is found with a center square and carefully marked and the hardness is measured at the center mark. Hardness measurements at any distance from the center of the core may be measured by drawing a line radially outward from the center mark, and measuring and marking the distance from the center, typically in 2-mm increments. All hardness measurements performed on the plane passing through the geometric

center are performed while the core is still in the holder and without having disturbed its orientation, such that the test surface is constantly parallel to the bottom of the holder. The hardness difference from any predetermined location on the core is calculated as the average surface hardness minus the hardness at the appropriate reference point, e.g., at the center of the core for single, solid core, such that a core surface softer than its center will have a negative hardness gradient.

Referring to TABLES 1-2, in Example 1, the surface is 10 Shore C points lower than the center hardness and 12 Shore C points lower than the hardest point in the core. In Example 3, the surface is 5 Shore C points lower than the center hardness and 8 Shore C points lower than the hardest point in the core. In Example 2, the center and surface hardness values are 15 equal and the softest point in the core is 10 Shore C points lower than the surface.

In the examples of the invention presented in TABLE 1, the cure temperatures are varied from 305° F. to 320° F. and cure times are varied from 11 to 16 minutes. The core compositions of examples 1 and 2 are identical, and only the cure cycle 20 is changed. In example 3 the amount of antioxidant is identical to examples 1 and 2, but other ingredients are varied as well the cure cycle. Additionally, the ratio of antioxidant to initiator varies from 0.50 to 0.57 from example 1 and 2 to 25 example 3.

The ratio of antioxidant to initiator is one factor to control the surface hardness of the cores. The data shown in TABLE 2 shows that hardness gradient is at least, but not limited to, a function of the amount of antioxidant and peroxide, their 30 ratio, and the cure cycle. It should be noted that higher antioxidant also requires higher peroxide initiator to maintain the desired compression.

The core of Comparative Example 1, whose composition is shown in TABLE 1 was cured using a conventional cure 35 cycle, with a cure temperature of 350° F. and a cure time of 11 minutes. The inventive cores were produced using cure cycles of 305° F. for 14 minutes, 315° F. for 11 minutes and 320° F. for 16 minutes. The hardness gradients of these cores were measured and the following observations can be made. For 40 the cores of the Comparative Examples, as expected, a conventional hard surface to soft center gradient can be clearly seen. The gradients for inventive cores follow substantially the same shape as one another.

In some embodiments of invention, the hardness of the core 45 at the surface is at most about the same as or substantially less than the hardness of the core at the center. Furthermore, the center hardness of the core may not be the hardest point in the core, but in these embodiments, it is preferred that it is at least equal to or harder than the surface. Additionally, the lowest 50 hardness anywhere in the core does not have to occur at the surface. In some embodiments, the lowest hardness value occurs within about the outer 6 mm of the core surface. However, the lowest hardness value within the core can occur at any point from the surface, up to, but not including the center, as long as the surface hardness is still equal to, or less 55 than the hardness of the center. It should be noted that in the present invention the formulation is the same throughout the core, or core layer, and no surface treatment is applied to the core to obtain the preferred surface hardness.

In FIG. 1, golf ball 2 comprises single layer core 4 and cover 6. The single layer core 4 comprises a geometric center 8 and outer surface 9. Outer surface 9 has been treated with and comprises a fatty acid/fatty acid salt composition. In FIG. 2, golf ball 10 comprises single layer core 12 and cover 4. 60 Single layer core 12 comprises a geometric center 16 and an outer surface 18. Single layer core 12 further comprises an untreated region 20 and treated region 22, the treated region

22 having been treated with and comprising a fatty acid/fatty acid salt composition. Untreated region 20 extends radially from geometric center 16 a distance  $D_{UT}$ , and is concentric with the geometric center 16. Treated region 22 is disposed about untreated region 20 and extends inward from outer surface 18 a depth  $D_{Tr}$ .

FIGS. 3A and 3B depict a single layer core golf ball of the present invention before and after treatment of the core outer surface with a fatty acid/fatty acid salt composition. In FIG. 3A, golf ball 24 comprises single layer core 26 and cover 28. The single layer core 26 comprises a geometric center 30 and outer surface 32. Single layer core 26 further comprises untreated regions A, B, C, D, and E. Untreated region A is in geometric center 30 and untreated region E is in outer surface 32. In FIG. 3B, single layer core 26 comprises untreated regions A, B, C, and D and treated region E'.

FIGS. 4A and 4B depict a multilayer core golf ball of the present invention before and after treatment of the core outer surface with a fatty acid/fatty acid salt composition. In FIG. 4A, golf ball 34 comprises dual layer core 48 and cover 40. Dual layer core 48 comprises first core layer 36 and second core layer 38. First core layer 36 is disposed about and concentric with geometric center 42. Second core layer 38 is disposed about first core layer 36 and adjacent cover 40. Dual layer core 48 further comprises untreated regions F, G, H, I, J and K. The first core layer 36 comprises untreated regions F-I and the second core layer 38 comprises untreated regions J-K. Further, First outer surface 44 of the first core layer 36 comprises untreated region I and second outer surface 46 of the second core layer 38 comprises untreated region K. FIG. 4B differs from FIG. 4A at least in that the first and second outer surfaces 44 and 46 comprise treated regions I' and K', respectively.

The following prophetic examples, represented in Table 3 below, illustrate several embodiments of the present invention consistent with FIGS. 1-4:

TABLE 3

| DISTANCE<br>FROM<br>GEO. CTR    | [SHORE C<br>HARDNESS<br>UNTREATED CORE] |    |     |    |    | [SHORE C<br>HARDNESS<br>TREATED CORE] |    |     |    |    |
|---------------------------------|-----------------------------------------|----|-----|----|----|---------------------------------------|----|-----|----|----|
|                                 | I                                       | II | III | IV | V  | I                                     | II | III | IV | V  |
| (mm)                            |                                         |    |     |    |    |                                       |    |     |    |    |
| 0                               | 74                                      | 65 | 60  | 74 | 58 | 74                                    | 65 | 60  | 74 | 58 |
| 5                               | 75                                      | 68 | 66  | 74 | 65 | 75                                    | 68 | 66  | 74 | 65 |
| 10                              | 76                                      | 73 | 72  | 74 | 72 | 76                                    | 73 | 72  | 74 | 72 |
| 1 <sup>st</sup> O.S.            | —                                       | —  | —   | —  | 80 | —                                     | —  | —   | —  | 74 |
| 15                              | 76                                      | 78 | 80  | 73 | 84 | 76                                    | 78 | 80  | 73 | 84 |
| 2 <sup>nd</sup> O.S.<br>or O.S. | 76                                      | 80 | 86  | 71 | 88 | 70                                    | 74 | 80  | 68 | 82 |

Table 3 reveals the hardnesses of 5 cores at certain distances from their respective geometric centers before and after treatment of each core outer surface (referred to in Table 3 as "O.S." [single layer core] and 2<sup>nd</sup> O.S. [dual layer core]) with a fatty acid and/or fatty acid salt composition. For example, Core I is a single layer core wherein the hardness of untreated outer surface O.S. is 76 Shore C and the hardness of treated outer surface O.S. is 70 Shore C. Accordingly, the hardness of the core outer surface is reduced by 6 Shore C. Meanwhile, the core hardness gradient from geometric center ("0 mm") to outer surface O.S. changes from +2 in untreated core I (positive hardness gradient, core outer surface harder) to -4 in treated core I (negative hardness gradient, core outer surface softer). The core hardness gradient from distance 5 mm to outer surface O.S. changes from +1 in the untreated core to -5 in the treated core. The core hardness gradients

from distances 10 mm and 15 mm to outer surface O.S. change from 0 (a zero hardness gradient) in the untreated core to -6 in the treated core.

In another embodiment, not shown in Table 3, treated core I of Table 3 is modified such that the hardness of treated outer surface O.S. is 74 Shore C rather than 70 Shore C. Accordingly, the core hardness gradient in treated core I from geometric center (0 mm) to outer surface O.S. lowers from a positive gradient of +2 (in untreated core I) to a zero gradient (hardness of geometric center and treated outer surface substantially similar or the same).

Next, as shown in Table 3, for treated core II, the positive gradients from distances 0 mm, 5 mm and 10 mm to outer surface O.S. are lower than those in untreated core II. Moreover, in treated core II, there is a negative hardness gradient from distance 15 mm to treated outer surface O.S. whereas that gradient is positive in untreated core II.

In treated core III of Table 3, the positive gradients from distances 0 mm, 5 mm and 10 mm to outer surface O.S. are lower than in untreated core III. Additionally, in treated core III, there is a zero hardness gradient (no hardness difference) from distance 15 mm to treated outer surface O.S., whereas in untreated core III, the hardness gradient is positive.

For treated core IV, a core is achieved having an over all greater negative hardness gradient from geometric center (0 mm) to treated outer surface O.S. than in untreated core IV. Additionally, treated core IV displays a greater negative hardness gradient from each of distances 5 mm, 10 mm and 15 mm to treated outer surface O.S.

Treated Core V of Table 3 is a dual layer core having first and second outer surfaces (1<sup>st</sup> O.S. and 2<sup>nd</sup> O.S., respectively), having been treated with and comprising a fatty acid/fatty acid salt composition. Table 3 displays lower hardness gradients from each of distances 0 mm, 5 mm and 10 mm to 1<sup>st</sup> O.S. of treated core V than for untreated core V. Meanwhile, Table 3 reveals a negative hardness gradient of -2 from distance 15 mm to 2<sup>nd</sup> O.S. in treated core V whereas the gradient in untreated core V for this distance is +4.

While the inventive golf ball may be formed from a variety of differing and conventional cover materials (both intermediate layer(s) and outer cover layer), preferred cover materials include, but are not limited to:

- (1) Polyurethanes, such as those prepared from polyols or polyamines and diisocyanates or polyisocyanates and/or their prepolymers, and those disclosed in U.S. Pat. Nos. 5,334,673 and 6,506,851;
- (2) Polyureas, such as those disclosed in U.S. Pat. Nos. 5,484,870 and 6,835,794; and
- (3) Polyurethane-urea hybrids, blends or copolymers comprising urethane or urea segments.

Suitable polyurethane compositions comprise a reaction product of at least one polyisocyanate and at least one curing agent. The curing agent can include, for example, one or more polyamines, one or more polyols, or a combination thereof.

The polyisocyanate can be combined with one or more polyols to form a prepolymer, which is then combined with the at least one curing agent. Thus, the polyols described herein are suitable for use in one or both components of the polyurethane material, i.e., as part of a prepolymer and in the curing agent. Suitable polyurethanes are described in U.S. Patent Application Publication No. 2005/0176523, which is incorporated by reference in its entirety.

Any polyisocyanate available to one of ordinary skill in the art is suitable for use according to the invention. Exemplary polyisocyanates include, but are not limited to, 4,4'-diphenylmethane diisocyanate (MDI); polymeric MDI; carbodiimide-modified liquid MDI; 4,4'-dicyclohexylmethane diisocyanate

(H<sub>12</sub>MDI); p-phenylene diisocyanate (PPDI); m-phenylene diisocyanate (MPDI); toluene diisocyanate (TDI); 3,3'-dimethyl-4,4'-biphenylene diisocyanate; isophorone diisocyanate; 1,6-hexamethylene diisocyanate (HDI); naphthalene diisocyanate; xylene diisocyanate; p-tetramethylxylene diisocyanate; m-tetramethylxylene diisocyanate; ethylene diisocyanate; propylene-1,2-diisocyanate; tetramethylene-1,4-diisocyanate; cyclohexyl diisocyanate; dodecane-1,12-diisocyanate; cyclobutane-1,3-diisocyanate; cyclohexane-1,3-diisocyanate; cyclohexane-1,4-diisocyanate; 1-isocyanato-3,3,5-trimethyl-5-isocyanatomethylcyclohexane; methyl cyclohexylene diisocyanate; triisocyanate of HDI; triisocyanate of 2,4,4-trimethyl-1,6-hexane diisocyanate; tetracene diisocyanate; naphthalene diisocyanate; anthracene diisocyanate; isocyanurate of toluene diisocyanate; uretdione of hexamethylene diisocyanate; and mixtures thereof. Polyisocyanates are known to those of ordinary skill in the art as having more than one isocyanate group, e.g., di-isocyanate, tri-isocyanate, and tetra-isocyanate. Preferably, the polyisocyanate includes MDI, PPDI, TDI, or a mixture thereof, and more preferably, the polyisocyanate includes MDI. It should be understood that, as used herein, the term MDI includes 4,4'-diphenylmethane diisocyanate, polymeric MDI, carbodiimide-modified liquid MDI, and mixtures thereof and, additionally, that the diisocyanate employed may be "low free monomer," understood by one of ordinary skill in the art to have lower levels of "free" monomer isocyanate groups, typically less than about 0.1% free monomer isocyanate groups. Examples of "low free monomer" diisocyanates include, but are not limited to Low Free Monomer MDI, Low Free Monomer TDI, and Low Free Monomer PPDI.

The at least one polyisocyanate should have less than about 14% unreacted NCO groups. Preferably, the at least one polyisocyanate has no greater than about 8.0% NCO, more preferably no greater than about 7.8%, and most preferably no greater than about 7.5% NCO with a level of NCO of about 7.2 or 7.0, or 6.5% NCO commonly used.

Any polyol available to one of ordinary skill in the art is suitable for use according to the invention. Exemplary polyols include, but are not limited to, polyether polyols, hydroxy-terminated polybutadiene (including partially/fully hydrogenated derivatives), polyester polyols, polycaprolactone polyols, and polycarbonate polyols. In one preferred embodiment, the polyol includes polyether polyol. Examples include, but are not limited to, polytetramethylene ether glycol (PTMEG), polyethylene propylene glycol, polyoxypolyethylene glycol, and mixtures thereof. The hydrocarbon chain can have saturated or unsaturated bonds and substituted or unsubstituted aromatic and cyclic groups. Preferably, the polyol of the present invention includes PTMEG.

In another embodiment, polyester polyols are included in the polyurethane material. Suitable polyester polyols include, but are not limited to, polyethylene adipate glycol; polybutylene adipate glycol; polyethylene propylene adipate glycol; o-phthalate-1,6-hexanediol; poly(hexamethylene adipate) glycol; and mixtures thereof. The hydrocarbon chain can have saturated or unsaturated bonds, or substituted or unsubstituted aromatic and cyclic groups.

In another embodiment, polycaprolactone polyols are included in the materials of the invention. Suitable polycaprolactone polyols include, but are not limited to, 1,6-hexanediol-initiated polycaprolactone, diethylene glycol initiated polycaprolactone, trimethylol propane initiated polycaprolactone, neopentyl glycol initiated polycaprolactone, 1,4-butanediol-initiated polycaprolactone, and mix-

tures thereof. The hydrocarbon chain can have saturated or unsaturated bonds, or substituted or unsubstituted aromatic and cyclic groups.

In yet another embodiment, polycarbonate polyols are included in the polyurethane material of the invention. Suitable polycarbonates include, but are not limited to, polyphthalate carbonate and poly(hexamethylene carbonate) glycol. The hydrocarbon chain can have saturated or unsaturated bonds, or substituted or unsubstituted aromatic and cyclic groups. In one embodiment, the molecular weight of the polyol is from about 200 to about 4000.

Polyamine curatives are also suitable for use in the polyurethane composition of the invention and have been found to improve cut, shear, and impact resistance of the resultant balls. Preferred polyamine curatives include, but are not limited to, 3,5-dimethylthio-2,4-toluenediamine and isomers thereof; 3,5-diethyltoluene-2,4-diamine and isomers thereof, such as 3,5-diethyltoluene-2,6-diamine; 4,4'-bis-(sec-butylamino)-diphenylmethane; 1,4-bis-(sec-butylamino)-benzene, 4,4'-methylene-bis-(2-chloroaniline); 4,4'-methylene-bis-(3-chloro-2,6-diethylaniline); polytetramethyleneoxide-di-p-aminobenzoate; N,N'-dialkyldiamino diphenyl methane; p,p'-methylene dianiline; m-phenylenediamine; 4,4'-methylene-bis-(2-chloroaniline); 4,4'-methylene-bis-(2,6-diethylaniline); 4,4'-methylene-bis-(2,3-dichloroaniline); 4,4'-diamino-3,3'-diethyl-5,5'-dimethyl diphenylmethane; 2,2',3,3'-tetrachloro diamino diphenylmethane; trimethylene glycol di-p-aminobenzoate; and mixtures thereof. Preferably, 30 the curing agent of the present invention includes 3,5-dimethylthio-2,4-toluenediamine and isomers thereof, such as ETHACURE® 300, commercially available from Albermarle Corporation of Baton Rouge, La. Suitable polyamine curatives, which include both primary and secondary amines, 35 preferably have molecular weights ranging from about 64 to about 2000.

At least one of a diol, triol, tetraol, or hydroxy-terminated curatives may be added to the aforementioned polyurethane composition. Suitable diol, triol, and tetraol groups include 40 ethylene glycol; diethylene glycol; polyethylene glycol; propylene glycol; polypropylene glycol; lower molecular weight polytetramethylene ether glycol; 1,3-bis(2-hydroxyethoxy)benzene; 1,3-bis-[2-(2-hydroxyethoxy)ethoxy]benzene; 1,3-bis-[2-[2-(2-hydroxyethoxy)ethoxy]ethoxy]benzene; 1,4-45 butanediol; 1,5-pentanediol; 1,6-hexanediol; resorcinol-di-(β-hydroxyethyl)ether; hydroquinone-di-(β-hydroxyethyl) ether; and mixtures thereof. Preferred hydroxy-terminated curatives include 1,3-bis(2-hydroxyethoxy)benzene; 1,3-bis-[2-(2-hydroxyethoxy)ethoxy]benzene; 1,3-bis-[2-[2-(2-hydroxyethoxy)ethoxy]ethoxy]benzene; 1,4-butanediol, and mixtures thereof. Preferably, the hydroxy-terminated curatives have molecular weights ranging from about 48 to 2000. It should be understood that molecular weight, as used herein, is the absolute weight average molecular weight and would be 50 understood as such by one of ordinary skill in the art.

Both the hydroxy-terminated and amine curatives can include one or more saturated, unsaturated, aromatic, and cyclic groups. Additionally, the hydroxy-terminated and amine curatives can include one or more halogen groups. The 55 polyurethane composition can be formed with a blend or mixture of curing agents. If desired, however, the polyurethane composition may be formed with a single curing agent.

In a preferred embodiment of the present invention, saturated polyurethanes are used to form one or more of the cover layers, preferably the outer cover layer, and may be selected 60 from among both castable thermoset and thermoplastic polyurethanes.

In this embodiment, the saturated polyurethanes of the present invention are substantially free of aromatic groups or moieties. Saturated polyurethanes suitable for use in the invention are a product of a reaction between at least one polyurethane prepolymer and at least one saturated curing agent. The polyurethane prepolymer is a product formed by a reaction between at least one saturated polyol and at least one saturated diisocyanate. As is well known in the art, that a catalyst may be employed to promote the reaction between the curing agent and the isocyanate and polyol, or the curing agent and the prepolymer.

Saturated diisocyanates which can be used include, without limitation, ethylene diisocyanate; propylene-1,2-diisocyanate; tetramethylene-1,4-diisocyanate; 1,6-hexamethylene-diisocyanate (HDI); 2,2,4-trimethylhexamethylene diisocyanate; 2,4,4-trimethylhexamethylene diisocyanate; dodecane-1,12-diisocyanate; dicyclohexylmethane diisocyanate; cyclobutane-1,3-diisocyanate; cyclohexane-1,3-diisocyanate; cyclohexane-1,4-diisocyanate; 1-isocyanato-3,3,5-trimethyl-5-isocyanatomethylcyclohexane; isophorone diisocyanate; methyl cyclohexylene diisocyanate; triisocyanate of HDI; triisocyanate of 2,2,4-trimethyl-1,6-hexane diisocyanate. The most preferred saturated diisocyanates are 4,4'-dicyclohexylmethane diisocyanate and isophorone diisocyanate.

Saturated polyols which are appropriate for use in this invention include without limitation polyether polyols such as polytetramethylene ether glycol and poly(oxypropylene) glycol. Suitable saturated polyester polyols include polyethylene adipate glycol, polyethylene propylene adipate glycol, polybutylene adipate glycol, polycarbonate polyol and ethylene oxide-capped polyoxypropylene diols. Saturated polycaprolactone polyols which are useful in the invention include diethylene glycol-initiated polycaprolactone, 1,4-butanediol-initiated polycaprolactone, 1,6-hexanediol-initiated polycaprolactone; trimethylol propane-initiated polycaprolactone, neopentyl glycol initiated polycaprolactone, and polytetramethylene ether glycol-initiated polycaprolactone. The most preferred saturated polyols are polytetramethylene ether glycol and PTMEG-initiated polycaprolactone.

Suitable saturated curatives include 1,4-butanediol, ethylene glycol, diethylene glycol, polytetramethylene ether glycol, propylene glycol; trimethanolpropane; tetra-(2-hydroxypropyl)-ethylenediamine; isomers and mixtures of isomers of cyclohexyldimethylol, isomers and mixtures of isomers of cyclohexane bis(methylamine); triisopropanolamine; ethylene diamine; diethylene triamine; triethylene tetramine; tetraethylene pentamine; 4,4'-dicyclohexylmethane diamine; 2,2,4-trimethyl-1,6-hexanediamine; 2,4,4-trimethyl-1,6-hexanediamine; diethyleneglycol di-(aminopropyl)ether; 4,4'-bis-(sec-butylamino)-dicyclohexylmethane; 1,2-bis-(sec-butylamino)cyclohexane; 1,4-bis-(sec-butylamino)cyclohexane; isophorone diamine; hexamethylene diamine; propylene diamine; 1-methyl-2,4-cyclohexyl diamine; 1-methyl-2,6-cyclohexyl diamine; 1,3-diaminopropane; dimethylamino propylamine; diethylamino propylamine; imido-bis-propylamine; isomers and mixtures of isomers of diaminocyclohexane; monoethanolamine; diethanolamine; triethanolamine; monoisopropanolamine; and diisopropanolamine. The most preferred saturated curatives are 1,4-butanediol, 1,4-cyclohexyldimethylol and 4,4'-bis-(sec-butylamino)-dicyclohexylmethane.

Alternatively, other suitable polymers include partially or fully neutralized ionomer, metallocene, or other single-site catalyzed polymer, polyester, polyamide, non-ionomeric thermoplastic elastomer, copolyether-esters, copolyether-amides, polycarbonate, polybutadiene, polyisoprene,

polystyrene block copolymers (such as styrene-butadiene-styrene), styrene-ethylene-propylene-styrene, styrene-ethylene-butylene-styrene, and the like, and blends thereof.

Thermosetting polyurethanes or polyureas are suitable for the outer cover layers of the golf balls of the present invention.

Additionally, polyurethane can be replaced with or blended with a polyurea material. Polyureas are distinctly different from polyurethane compositions, but also result in desirable aerodynamic and aesthetic characteristics when used in golf ball components. The polyurea-based compositions are preferably saturated in nature.

Without being bound to any particular theory, it is now believed that substitution of the long chain polyol segment in the polyurethane prepolymer with a long chain polyamine oligomer soft segment to form a polyurea prepolymer, improves shear, cut, and resiliency, as well as adhesion to other components. Thus, the polyurea compositions of this invention may be formed from the reaction product of an isocyanate and polyamine prepolymer crosslinked with a curing agent. For example, polyurea-based compositions of the invention may be prepared from at least one isocyanate, at least one polyether amine, and at least one diol curing agent or at least one diamine curing agent.

Any polyamine available to one of ordinary skill in the art is suitable for use in the polyurea prepolymer. Polyether amines are particularly suitable for use in the prepolymer. As used herein, "polyether amines" refer to at least polyoxyalkyleneamines containing primary amino groups attached to the terminus of a polyether backbone. Due to the rapid reaction of isocyanate and amine, and the insolubility of many urea products, however, the selection of diamines and polyether amines is limited to those allowing the successful formation of the polyurea prepolymers. In one embodiment, the polyether backbone is based on tetramethylene, propylene, ethylene, trimethylolpropane, glycerin, and mixtures thereof.

Suitable polyether amines include, but are not limited to, methyldiethanolamine; polyoxyalkylenediamines such as, polytetramethylene ether diamines, polyoxypropylenetriamine, and polyoxypropylene diamines; poly(ethylene oxide) capped oxypropylene)ether diamines; propylene oxide-based triamines; triethyleneglycoldiamines; trimethylolpropane-based triamines; glycerin-based triamines; and mixtures thereof. In one embodiment, the polyether amine used to form the prepolymer is JEFFAMINE® D2000 (manufactured by Huntsman Chemical Co. of Austin, Tex.).

The molecular weight of the polyether amine for use in the polyurea prepolymer may range from about 100 to about 5000. In one embodiment, the polyether amine molecular weight is about 200 or greater, preferably about 230 or greater. In another embodiment, the molecular weight of the polyether amine is about 4000 or less. In yet another embodiment, the molecular weight of the polyether amine is about 600 or greater. In still another embodiment, the molecular weight of the polyether amine is about 3000 or less. In yet another embodiment, the molecular weight of the polyether amine is between about 1000 and about 3000, and more preferably is between about 1500 to about 2500. Because lower molecular weight polyether amines may be prone to forming solid polyureas, a higher molecular weight oligomer, such as JEFFAMINE® D2000, is preferred.

As briefly discussed above, some amines may be unsuitable for reaction with the isocyanate because of the rapid reaction between the two components. In particular, shorter chain amines are fast reacting. In one embodiment, however, a hindered secondary diamine may be suitable for use in the prepolymer. Without being bound to any particular theory, it is believed that an amine with a high level of stearic hin-

drance, e.g., a tertiary butyl group on the nitrogen atom, has a slower reaction rate than an amine with no hindrance or a low level of hindrance. For example, 4,4'-bis-(sec-butylamino)-dicyclohexylmethane (CLEARLINK® 1000) may be suitable for use in combination with an isocyanate to form the polyurea prepolymer.

Any isocyanate available to one of ordinary skill in the art is suitable for use in the polyurea prepolymer. Isocyanates for use with the present invention include aliphatic, cycloaliphatic, araliphatic, aromatic, any derivatives thereof, and combinations of these compounds having two or more isocyanate (NCO) groups per molecule. The isocyanates may be organic polyisocyanate-terminated prepolymers. The isocyanate-containing reactable component may also include any isocyanate-functional monomer, dimer, trimer, or multi-meric adduct thereof, prepolymer, quasi-prepolymer, or mixtures thereof. Isocyanate-functional compounds may include monoisocyanates or polyisocyanates that include any isocyanate functionality of two or more.

Suitable isocyanate-containing components include diisocyanates having the generic structure:  $O=C=N-R-N=C=O$ , where R is preferably a cyclic, aromatic, or linear or branched hydrocarbon moiety containing from about 1 to about 20 carbon atoms. The diisocyanate may also contain one or more cyclic groups or one or more phenyl groups. When multiple cyclic or aromatic groups are present, linear and/or branched hydrocarbons containing from about 1 to about 10 carbon atoms can be present as spacers between the cyclic or aromatic groups. In some cases, the cyclic or aromatic group(s) may be substituted at the 2-, 3-, and/or 4-positions, or at the ortho-, meta-, and/or para-positions, respectively. Substituted groups may include, but are not limited to, halogens, primary, secondary, or tertiary hydrocarbon groups, or a mixture thereof.

Examples of diisocyanates that can be used with the present invention include, but are not limited to, substituted and isomeric mixtures including 2,2'-, 2,4'-, and 4,4'-diphenylmethane diisocyanate; 3,3'-dimethyl-4,4'-biphenylene diisocyanate; toluene diisocyanate; polymeric MDI; carbodi-imide-modified liquid 4,4'-diphenylmethane diisocyanate; para-phenylene diisocyanate; meta-phenylene diisocyanate; triphenyl methane-4,4'- and triphenyl methane-4,4'-triisocyanate; naphthylene-1,5-diisocyanate; 2,4'-, 4,4'-, and 2,2-biphenyl diisocyanate; polyphenyl polymethylene polyisocyanate; mixtures of MDI and PMDI; mixtures of PMDI and TDI; ethylene diisocyanate; propylene-1,2-diisocyanate; tetramethylene-1,2-diisocyanate; tetramethylene-1,3-diisocyanate; tetramethylene-1,4-diisocyanate; 1,6-hexamethylene-diisocyanate; octamethylene diisocyanate; decamethylene diisocyanate; 2,2,4-trimethylhexamethylene diisocyanate; 2,4,4-trimethylhexamethylene diisocyanate; dodecane-1,12-diisocyanate; cyclobutane-1,3-diisocyanate; cyclohexane-1,2-diisocyanate; cyclohexane-1,3-diisocyanate; cyclohexane-1,4-diisocyanate; methyl-cyclohexylene diisocyanate; 2,4-methylcyclohexane diisocyanate; 2,6-methylcyclohexane diisocyanate; 4,4'-dicyclohexyl diisocyanate; 2,4'-dicyclohexyl diisocyanate; 1,3,5-cyclohexane triisocyanate; isocyanatomethylcyclohexane isocyanate; 1-isocyanato-3,3,5-trimethyl-5-isocyanatomethylcyclohexane; isocyanatoethylcyclohexane isocyanate; bis(isocyanatomethyl)-cyclohexane diisocyanate; 4,4'-bis(isocyanatomethyl) dicyclohexane; 4,4'-bis(isocyanatomethyl) dicyclohexane; isophorone diisocyanate; triisocyanate of HDI; triisocyanate of 2,2,4-trimethyl-1,6-hexane diisocyanate; 4,4'-dicyclohexylmethane diisocyanate; 2,4-hexahydrotoluene diisocyanate; 2,6-hexahydrotoluene diisocyanate; and mixtures thereof. Aromatic aliphatic isocyanates may also be used to form light stable materials. Examples of such isocyanates include 1,2-, 1,3-, and 1,4-xylene diisocyanate; meta-tetramethylxylene diisocyanate; para-tetramethylxylene diisocyanate; trimerized isocyanurate of any polyisocyanate, such as isocyanurate of toluene diisocyanate, trimer of diphenylmethane diisocyanate, trimer of tetramethylxylene diisocyanate, isocyanurate of hexamethylene diisocyanate, isocyanurate of isophorone diisocyanate, and mixtures thereof; dimerized uredione of any polyisocyanate, such as uredione of toluene diisocyanate, uredione of hexamethylene diisocyanate, and mixtures thereof; modified polyisocyanate derived from the above isocyanates and polyisocyanates; and mixtures thereof.

Examples of saturated diisocyanates that can be used with the present invention include, but are not limited to, ethylene diisocyanate; propylene-1,2-diisocyanate; tetramethylene diisocyanate; tetramethylene-1,4-diisocyanate; 1,6-hexamethylene-diisocyanate; octamethylene diisocyanate; decamethylene diisocyanate; 2,2,4-trimethylhexamethylene diisocyanate; 2,4,4-trimethylhexamethylene diisocyanate; dodecane-1,12-diisocyanate; cyclobutane-1,3-diisocyanate; cyclohexane-1,2-diisocyanate; cyclohexane-1,3-diisocyanate; cyclohexane-1,4-diisocyanate; methyl-cyclohexylene diisocyanate; 2,4-methylcyclohexane diisocyanate; 2,6-methylcyclohexane diisocyanate; 4,4'-dicyclohexyl diisocyanate; 2,4'-dicyclohexyl diisocyanate; 1,3,5-cyclohexane triisocyanate; isocyanatomethylcyclohexane isocyanate; 1-isocyanato-3,3,5-trimethyl-5-isocyanatomethylcyclohexane; isocyanatoethylcyclohexane isocyanate; bis(isocyanatomethyl)-cyclohexane diisocyanate; 4,4'-bis(isocyanatomethyl) dicyclohexane; 4,4'-bis(isocyanatomethyl) dicyclohexane; isophorone diisocyanate; triisocyanate of HDI; triisocyanate of 2,2,4-trimethyl-1,6-hexane diisocyanate; 4,4'-dicyclohexylmethane diisocyanate; 2,4-hexahydrotoluene diisocyanate; 2,6-hexahydrotoluene diisocyanate; and mixtures thereof. Aromatic aliphatic isocyanates may also be used to form light stable materials. Examples of such isocyanates include 1,2-, 1,3-, and 1,4-xylene diisocyanate; meta-tetramethylxylene diisocyanate; para-tetramethylxylene diisocyanate; trimerized isocyanurate of any polyisocyanate, such as isocyanurate of toluene diisocyanate, trimer of diphenylmethane diisocyanate, trimer of tetramethylxylene diisocyanate, isocyanurate of hexamethylene diisocyanate, isocyanurate of isophorone diisocyanate, and mixtures thereof; dimerized uredione of any polyisocyanate, such as uredione of toluene diisocyanate, uredione of hexamethylene diisocyanate, and mixtures thereof; modified polyisocyanate derived from the above isocyanates and polyisocyanates; and mixtures thereof.

The number of unreacted NCO groups in the polyurea prepolymer of isocyanate and polyether amine may be varied to control such factors as the speed of the reaction, the resultant hardness of the composition, and the like. For instance, the number of unreacted NCO groups in the polyurea prepolymer of isocyanate and polyether amine may be less than about 14 percent. In one embodiment, the polyurea prepolymer has from about 5 percent to about 11 percent unreacted NCO groups, and even more preferably has from about 6 to about 9.5 percent unreacted NCO groups. In one embodiment, the percentage of unreacted NCO groups is about 3 percent to about 9 percent. Alternatively, the percentage of unreacted NCO groups in the polyurea prepolymer may be about 7.5 percent or less, and more preferably, about 7 percent or less. In another embodiment, the unreacted NCO content is from about 2.5 percent to about 7.5 percent, and more preferably from about 4 percent to about 6.5 percent.

When formed, polyurea prepolymers may contain about 10 percent to about 20 percent by weight of the prepolymer of free isocyanate monomer. Thus, in one embodiment, the polyurea prepolymer may be stripped of the free isocyanate monomer. For example, after stripping, the prepolymer may contain about 1 percent or less free isocyanate monomer. In another embodiment, the prepolymer contains about 0.5 percent by weight or less of free isocyanate monomer.

The polyether amine may be blended with additional polyols to formulate copolymers that are reacted with excess isocyanate to form the polyurea prepolymer. In one embodiment, less than about 30 percent polyol by weight of the copolymer is blended with the saturated polyether amine. In another embodiment, less than about 20 percent polyol by weight of the copolymer, preferably less than about 15 percent by weight of the copolymer, is blended with the polyether amine. The polyols listed above with respect to the polyurethane prepolymer, e.g., polyether polyols, polycaprolactone polyols, polyester polyols, polycarbonate polyols, hydrocarbon polyols, other polyols, and mixtures thereof, are also suitable for blending with the polyether amine. The molecular weight of these polymers may be from about 200 to about 4000, but also may be from about 1000 to about 3000, and more preferably are from about 1500 to about 2500.

The polyurea composition can be formed by crosslinking the polyurea prepolymer with a single curing agent or a blend of curing agents. The curing agent of the invention is preferably an amine-terminated curing agent, more preferably a secondary diamine curing agent so that the composition contains only ureal linkages. In one embodiment, the amine-terminated curing agent may have a molecular weight of about 64 or greater. In another embodiment, the molecular weight of the amine-curing agent is about 2000 or less. As discussed above, certain amine-terminated curing agents may be modified with a compatible amine-terminated freezing point depressing agent or mixture of compatible freezing point depressing agents.

Suitable amine-terminated curing agents include, but are not limited to, ethylene diamine; hexamethylene diamine; 1-methyl-2,6-cyclohexyl diamine; tetrahydroxypropylene ethylene diamine; 2,2,4- and 2,4,4-trimethyl-1,6-hexanediamine; 4,4'-bis-(sec-butylamino)-dicyclohexylmethane; 1,4-bis-(sec-butylamino)-cyclohexane; 1,2-bis-(sec-butylamino)-cyclohexane; derivatives of 4,4'-bis-(sec-butylamino)-dicyclohexylmethane; 4,4'-dicyclohexylmethane diamine; 1,4-cyclohexane-bis-(methylamine); 1,3-cyclohexane-bis-(methylamine); diethylene glycol di-(aminopropyl)ether; 2-methylpentamethylene-diamine; diaminocyclohexane; diethylene triamine; triethylene tetramine; tetraethylene pentamine; propylene diamine; 1,3-diaminopropane; dimethylamino propylamine; diethylamino propylamine; dipropylene triamine; imido-bis-propylamine; monoethanolamine, diethanolamine; triethanolamine; monoisopropanolamine, diisopropanolamine; isophoronediamine; triisopropanolamine; and mixtures thereof. In one

embodiment, the amine-terminated curing agent is 4,4'-bis-(sec-butylamino)-dicyclohexylmethane.

Suitable saturated amine-terminated curing agents include, but are not limited to, ethylene diamine; hexamethylene diamine; 1-methyl-2,6-cyclohexyl diamine; tetrahydroxypropylene ethylene diamine; 2,2,4- and 2,4,4-trimethyl-1,6-hexanediamine; 4,4'-bis-(sec-butylamino)-dicyclohexylmethane; 1,4-bis-(sec-butylamino)-cyclohexane; 1,2-bis-(sec-butylamino)-cyclohexane; derivatives of 4,4'-bis-(sec-butylamino)-dicyclohexylmethane; 4,4'-dicyclohexylmethane diamine; 4,4'-methylenebis-(2,6-diethylaminocyclohexane); 1,4-cyclohexane-bis-(methylamine); 1,3-cyclohexane-bis-(methylamine); diethylene glycol di-(aminopropyl)ether; 2-methylpentamethylene-diamine; diaminocyclohexane; diethylene triamine; triethylene tetramine; tetraethylene pentamine; propylene diamine; 1,3-diaminopropane; dimethylamino propylamine; diethylamino propylamine; imido-bis-propylamine; monoethanolamine, diethanolamine; triethanolamine; monoisopropanolamine, diisopropanolamine; isophoronediamine; triisopropanolamine; and mixtures thereof. In addition, any of the polyether amines listed above may be used as curing agents to react with the polyurea prepolymers.

Cover layers of the inventive golf ball may also be formed from ionomeric polymers, preferably highly-neutralized ionomers (HNP). In a preferred embodiment, at least one intermediate layer of the golf ball is formed from an HNP material or a blend of HNP materials. The acid moieties of the HNP's, typically ethylene-based ionomers, are preferably neutralized greater than about 70%, more preferably greater than about 90%, and most preferably at least about 100%. The HNP's can be also be blended with a second polymer component, which, if containing an acid group, may be neutralized in a conventional manner, by the organic fatty acids of the present invention, or both. The second polymer component, which may be partially or fully neutralized, preferably comprises ionomeric copolymers and terpolymers, ionomer precursors, thermoplastics, polyamides, polycarbonates, polyesters, polyurethanes, polyureas, thermoplastic elastomers, polybutadiene rubber, balata, metallocene-catalyzed polymers (grafted and non-grafted), single-site polymers, high-crystalline acid polymers, cationic ionomers, and the like. HNP polymers typically have a material hardness of between about 20 and about 80 Shore D, and a flexural modulus of between about 3,000 psi and about 200,000 psi.

In one embodiment of the present invention the HNP's are ionomers and/or their acid precursors that are preferably neutralized, either fully or partially, with organic acid copolymers or the salts thereof. The acid copolymers are preferably  $\alpha$ -olefin, such as ethylene,  $C_{3-8}$   $\alpha,\beta$ -ethylenically unsaturated carboxylic acid, such as acrylic and methacrylic acid, copolymers. They may optionally contain a softening monomer, such as alkyl acrylate and alkyl methacrylate, wherein the alkyl groups have from 1 to 8 carbon atoms.

The acid copolymers can be described as E/X/Y copolymers where E is ethylene, X is an  $\alpha,\beta$ -ethylenically unsaturated carboxylic acid, and Y is a softening comonomer. In a preferred embodiment, X is acrylic or methacrylic acid and Y is a  $C_{1-8}$  alkyl acrylate or methacrylate ester. X is preferably present in an amount from about 1 to about 35 weight percent of the polymer, more preferably from about 5 to about 30 weight percent of the polymer, and most preferably from about 10 to about 20 weight percent of the polymer. Y is preferably present in an amount from about 0 to about 50 weight percent of the polymer, more preferably from about 5 to about 25 weight percent of the polymer, and most preferably from about 10 to about 20 weight percent of the polymer.

Specific acid-containing ethylene copolymers include, but are not limited to, ethylene/acrylic acid/n-butyl acrylate, ethylene/methacrylic acid/n-butyl acrylate, ethylene/methacrylic acid/iso-butyl acrylate, ethylene/acrylic acid/iso-butyl acrylate, ethylene/methacrylic acid/n-butyl methacrylate, ethylene/acrylic acid/methyl methacrylate, ethylene/acrylic acid/methyl acrylate, ethylene/methacrylic acid/methyl acrylate, ethylene/acrylic acid/methyl methacrylate, and ethylene/acrylic acid/n-butyl methacrylate. Preferred acid-containing ethylene copolymers include, ethylene/methacrylic acid/n-butyl acrylate, ethylene/acrylic acid/n-butyl acrylate, ethylene/methacrylic acid/methyl acrylate, ethylene/acrylic acid/ethyl acrylate, ethylene/methacrylic acid/ethyl acrylate, and ethylene/acrylic acid/methyl acrylate copolymers. The most preferred acid-containing ethylene copolymers are, ethylene/(meth) acrylic acid/n-butyl acrylate, ethylene/(meth) acrylic acid/ethyl acrylate, and ethylene/(meth) acrylic acid/methyl acrylate copolymers.

Ionomers are typically neutralized with a metal cation, such as Li, Na, Mg, K, Ca, or Zn. It has been found that by adding sufficient organic acid or salt of organic acid, along with a suitable base, to the acid copolymer or ionomer, however, the ionomer can be neutralized, without losing processability, to a level much greater than for a metal cation. Preferably, the acid moieties are neutralized greater than about 80%, preferably from 90-100%, most preferably 100% without losing processability. This accomplished by melt-blending an ethylene  $\alpha,\beta$ -ethylenically unsaturated carboxylic acid copolymer, for example, with an organic acid or a salt of organic acid, and adding a sufficient amount of a cation source to increase the level of neutralization of all the acid moieties (including those in the acid copolymer and in the organic acid) to greater than 90%, (preferably greater than 100%).

The organic acids of the present invention are aliphatic, mono- or multi-functional (saturated, unsaturated, or multi-unsaturated) organic acids. Salts of these organic acids may also be employed. The salts of organic acids of the present invention include the salts of barium, lithium, sodium, zinc, bismuth, chromium, cobalt, copper, potassium, strontium, titanium, tungsten, magnesium, cesium, iron, nickel, silver, aluminum, tin, or calcium, salts of fatty acids, particularly stearic, behenic, erucic, oleic, linoleic or dimerized derivatives thereof. It is preferred that the organic acids and salts of the present invention be relatively non-migratory (they do not bloom to the surface of the polymer under ambient temperatures) and non-volatile (they do not volatilize at temperatures required for melt-blending).

The ionomers of the invention may also be more conventional ionomers, i.e., partially-neutralized with metal cations. The acid moiety in the acid copolymer is neutralized about 1 to about 90%, preferably at least about 20 to about 75%, and more preferably at least about 40 to about 70%, to form an ionomer, by a cation such as lithium, sodium, potassium, magnesium, calcium, barium, lead, tin, zinc, aluminum, or a mixture thereof.

In one embodiment, the inventive single-layer core is enclosed with two cover layers, where the inner cover layer has a thickness of about 0.01 inches to about 0.06 inches, more preferably about 0.015 inches to about 0.040 inches, and most preferably about 0.02 inches to about 0.035 inches, and the inner cover layer is formed from a partially- or fully-neutralized ionomer having a Shore D hardness of greater than about 55, more preferably greater than about 60, and most preferably greater than about 65. In this embodiment, the outer cover layer should have a thickness of about 0.015 inches to about 0.055 inches, more preferably about 0.02

inches to about 0.04 inches, and most preferably about 0.025 inches to about 0.035 inches, and has a hardness of about Shore D 60 or less, more preferably 55 or less, and most preferably about 52 or less. The inner cover layer should be harder than the outer cover layer. In this embodiment the outer cover layer comprises a partially- or fully-neutralized ionomer, a polyurethane, polyurea, or blend thereof. A most preferred outer cover layer is a castable or reaction injection molded polyurethane, polyurea or copolymer or hybrid thereof having a Shore D hardness of about 40 to about 50. A most preferred inner cover layer material is a partially-neutralized ionomer comprising a zinc, sodium or lithium neutralized ionomer such as SURLYN® 8940, 8945, 9910, 7930, 7940, or blend thereof having a Shore D hardness of about 63 to about 68.

In another multi-layer cover, single core embodiment, the outer cover and inner cover layer materials and thickness are the same but, the hardness range is reversed, that is, the outer cover layer is harder than the inner cover layer.

In an alternative embodiment, the golf ball is a one-piece golf ball having a dimpled surface and having a surface hardness equal to or less than the center hardness (i.e., a negative hardness gradient). The one-piece ball preferably has a diameter of about 1.680 inches to about 1.690 inches, a weight of about 1.620 oz, an Atti compression of from about 40 to 120, and a COR of about 0.750-0.825.

In a two-piece ball embodiment, the single-layer core having a negative hardness gradient is enclosed with a single layer of cover material having a Shore D hardness of from about 20 to about 80, more preferably about 40 to about 75 and most preferably about 45 to about 70, and comprises a thermoplastic or thermosetting polyurethane, polyurea, polyamide, polyester, polyester elastomer, polyether-amide or polyester-amide, partially or fully neutralized ionomer, polyolefin such as polyethylene, polypropylene, polyethylene copolymers such as ethylene-butyl acrylate or ethylene-methyl acrylate, poly(ethylene methacrylic acid) co- and terpolymers, metallocene-catalyzed polyolefins and polar-group functionalized polyolefins and blends thereof. A preferred cover material in the two-piece embodiment is an ionomer (either conventional or HNP) having a hardness of about 50 to about 70 Shore D. Another preferred cover material in the two-piece embodiment is a thermoplastic or thermosetting polyurethane or polyurea. A preferred ionomer is a high acid ionomer comprising a copolymer of ethylene and methacrylic or acrylic acid and having an acid content of at least 16 to about 25 weight percent. In this case the reduced spin contributed by the relatively rigid high acid ionomer may be offset to some extent by the spin-increasing negative gradient core. The core may have a diameter of about 1.0 inch to about 1.64 inches, preferably about 1.30 inches to about 1.620, and more preferably about 1.40 inches to about 1.60 inches.

Another preferred cover material comprises a castable or reaction injection moldable polyurethane, polyurea, or copolymer or hybrid of polyurethane/polyurea. Preferably, this cover is thermosetting but may be a thermoplastic, having a Shore D hardness of about 20 to about 70, more preferably about 30 to about 65 and most preferably about 35 to about 60.

A moisture vapor barrier layer, such as disclosed in U.S. Pat. Nos. 6,632,147; 6,932,720; 7,004,854; and 7,182,702, all of which are incorporated by reference herein in their entirety, are optionally employed between the cover layer and the core.

While any of the embodiments herein may have any known dimple number and pattern, a preferred number of dimples is 252 to 456, and more preferably is 330 to 392. The dimples may comprise any width, depth, and edge angle disclosed in

the prior art and the patterns may comprises multitudes of dimples having different widths, depths and edge angles. The parting line configuration of said pattern may be either a straight line or a staggered wave parting line (SWPL). Most preferably the dimple number is 330, 332, or 392 and comprises 5 to 7 dimples sizes and the parting line is a SWPL.

In any of these embodiments the single-layer core may be replaced with a 2 or more layer core wherein at least one core layer has a negative hardness gradient.

Other than in the operating examples, or unless otherwise expressly specified, all of the numerical ranges, amounts, values and percentages such as those for amounts of materials and others in the specification may be read as if prefaced by the word "about" even though the term "about" may not expressly appear with the value, amount or range. Accordingly, unless indicated to the contrary, the numerical parameters set forth in the specification and attached claims are approximations that may vary depending upon the desired properties sought to be obtained by the present invention. At the very least, and not as an attempt to limit the application of the doctrine of equivalents to the scope of the claims, each numerical parameter should at least be construed in light of the number of reported significant digits and by applying ordinary rounding techniques.

Notwithstanding that the numerical ranges and parameters setting forth the broad scope of the invention are approximations, the numerical values set forth in the specific examples are reported as precisely as possible. Any numerical value, however, inherently contain certain errors necessarily resulting from the standard deviation found in their respective testing measurements. Furthermore, when numerical ranges of varying scope are set forth herein, it is contemplated that any combination of these values inclusive of the recited values may be used. While it is apparent that the illustrative embodiments of the invention disclosed herein fulfill the objective stated above, it is appreciated that numerous modifications and other embodiments may be devised by those skilled in the art. Therefore, it will be understood that the appended claims are intended to cover all such modifications and embodiments, which would come within the spirit and scope of the present invention.

What is claimed is:

1. A golf ball comprising a core and a cover, said core comprising an outer surface and a geometric center, the outer surface being treated with and comprising a fatty acid and/or fatty acid salt composition, the outer surface further having a first hardness and the geometric center having a second hardness, wherein the first hardness is less than the second hardness to define a negative hardness gradient.

2. The golf ball of claim 1, wherein the core comprises a 50 thermoset rubber composition.

3. The golf ball of claim 2, wherein the thermoset rubber composition comprises a polybutadiene material and the core comprises a surface hardness of about 50 Shore C or greater.

4. The golf ball of claim 3, wherein the polybutadiene composition is at least partially crosslinked.

5. The golf ball of claim 1, wherein the fatty acid and/or fatty acid salt composition comprises oleic acid, palmitic acid, stearic acid, behenic acid, pelargonic acid, linoleic acid,

linolenic acid, arachidonic acid, caproic acid, caprylic acid, capric acid, lauric acid, erucic acid, myristic acid, benzoic acid, phenylacetic acid, or naphthalenoic acid.

6. The golf ball of claim 5, wherein the fatty acid and/or fatty acid salt composition comprises a cation selected from the group comprising barium, lithium, sodium, zinc, bismuth, chromium, cobalt, copper, potassium, strontium, titanium, tungsten, magnesium, cesium, iron, nickel, silver, aluminum, tin and calcium.

7. The golf ball of claim 1, wherein the fatty acid and/or fatty acid salt composition further comprises at least one of an antioxidant, a peroxide, a sulfur-bearing compound, zinc methacrylate, zinc dimethacrylate, a softening acrylate monomer or oligomer, a thermoplastic resin, or an hydroquinone.

8. The golf ball of claim 7, wherein the thermoplastic resin comprises at least one of polyethylene vinyl acetate, polyethylene butyl acrylate, polyethylene methyl acrylate, polyethylene acrylic acid, polyethylene methacrylic acid or an ionomer.

9. The golf ball of claim 1, further comprising an intermediate core layer disposed about the core and adjacent the cover layer.

10. A golf ball comprising a core and a cover, said core comprising an outer surface and a geometric center, wherein the outer surface comprises a fatty acid and/or fatty acid salt composition and has a first hardness and the geometric center does not comprise the fatty acid and/or fatty acid salt composition and has a second hardness greater than the first hardness to define a negative hardness gradient.

11. A golf ball comprising a core and a cover, wherein the core comprises a geometric center and a treated outer surface, the treated outer surface having a first hardness and the geometric center having a second hardness, the treated outer surface being treated with a surface-softening material comprising at least one fatty acid and/or fatty acid salt composition such that the second hardness is greater than the first hardness to define a negative hardness gradient.

12. A golf ball comprising a core and a cover, said core comprising a fatty acid and/or fatty acid salt composition outer surface and a geometric center that does not comprise the fatty acid and/or fatty acid salt composition, the fatty acid and/or fatty acid salt composition outer surface having a first hardness and the geometric center having a second hardness wherein the first hardness is less than the second hardness to define a negative hardness gradient.

13. The golf ball of claim 12, wherein the core comprises a thermoset rubber composition.

14. A golf ball comprising a core and a cover, said core comprising an outer surface and a geometric center, the outer surface being treated with and comprising a fatty acid and/or fatty acid salt composition and having a first hardness, the geometric center not comprising the fatty acid and/or fatty acid salt composition and having a second hardness that is different than the first hardness.